# EUROPEAN PATENT SPECIFICATION

(11) **EP 3 505 655 B1**
(45) Date of publication and mention of the grant of the patent: **11.08.2021**
(21) Application number: 17842888.4
(22) Date of filing: 22.08.2017
(51) Int. Cl.: C23C 22/36, C23C 22/44, C23C 22/73, C23C 22/68, C23C 22/74

(54) **INORGANIC SURFACE-TREATED GALVANIZED STEEL SHEET, PREPARATION METHOD THEREFOR, AND AQUEOUS INORGANIC SURFACE TREATMENT AGENT THEREOF**
ANORGANISCHES OBERFLÄCHENBEHANDELTES VERZINKTES STAHLBLECH, HERSTELLUNGSVERFAHREN DAFÜR UND WÄSSRIGES ANORGANISCHES OBERFLÄCHENBEHANDLUNGSMITTEL DARAUS
FEUILLE D'ACIER GALVANISÉE TRAITÉE EN SURFACE INORGANIQUE, SON PROCÉDÉ DE PRÉPARATION, ET AGENT DE TRAITEMENT DE SURFACE INORGANIQUE AQUEUX ASSOCIÉ

(30) Priority: 24.08.2016 CN 201610719583
(43) Date of publication of application: 03.07.2019
(73) Proprietor: Baoshan Iron & Steel Co., Ltd., Shanghai 201900 (CN)
(72) Inventor: ZHANG, Jianping, Shanghai 201900 (CN); ZHANG, Wenqi, Shanghai 201900 (CN); DAI, Yigang, Shanghai 201900 (CN)
(74) Representative: Kuhnen & Wacker Patent- und Rechtsanwaltsbüro PartG mbB
(86) International application number: PCT/CN2017/098430
(87) International publication number: WO 2018/036465

(56) References cited:
- EP-A1- 2 957 657
- CN-A- 1 360 644
- CN-A- 101 899 657
- CN-A- 103 289 565
- CN-A- 104 629 603
- CN-A- 105 255 338
- CN-A- 105 255 338
- CN-A- 105 463 436

## Description

### Technical Field

The present invention pertains to the technical field of surface treatment of galvanized steel sheets. In particular, the present invention relates to an inorganically surface-treated galvanized steel sheet, a method of preparing the same and an aqueous inorganic surface treatment agent. The inorganically surface-treated galvanized steel sheet and the method of preparing the same can meet the requirements of rapid deep-drawing processing with progressive dies in the field of electrical micro-machines, and impart both excellent red rust resistance and surface electric conductivity to parts.

### Background Art

Galvanized steel sheets are widely used in various fields such as automobiles, home appliances, architectures, etc, and mostly used for parts of automobiles, home appliances, electrical micro-machines, etc. Meanwhile, as the degree of mechanical automation increases, various electrical micro-machines are widely used in automobiles, processing machines or electrical equipment.

However, due to the special requirements of processing and service of electrical micro-machines, a number of critical issues need attention in storage, transportation, processing and service of galvanized steel sheets for electrical micro-machines.

In order to prevent generation of white rust due to occurrence of tarnishing in transportation and storage of galvanized steel sheets, coating of rust preventive oil is needed in manufacture of the steel sheets. When stamping processing is performed with progressive dies in the field of electrical micro-machines, the stamping process of rapid deep drawing exasperates the frictional wear between the dies and the metallic sheets. To prevent cracking of the sheets and scratching of surface zinc layers, it's necessary to add lubricating oil to the dies when parts are stamped, after which the parts are degreased and washed. In the service of an electrical micro-machine, to guarantee the service life, grounding safety and electromagnetic characteristics of the electrical micro-machine, very high requirements are imposed on the red rust resistance and surface electric conductivity of stamped parts. The red rust resistance corresponds to the service life of the electrical micro-machine, and the surface electric conductivity corresponds to the grounding safety and the electromagnetic characteristics of the electrical micro-machine. First of all, the use of the rust preventive oil, lubricating oil and degreasing agent throughout the storage and stamping of the galvanized steel sheets is undesirable for environment and production cost.

In order to improve corrosion resistance and formability, an existing method mainly involves surface treatment of a galvanized steel sheet by passivation with chromic acid. This method can improve the corrosion resistance of the steel sheet, but has limited improvement in formability and other resistances. It is not able to meet the requirements of rapid deep drawing with progressive dies in the field of electrical micro-machines. Alternatively, after passivation with a chromate salt, the steel sheet may be further coated with an organic resin comprising a solid lubricating aid (usually a low surface energy polymer such as polyolefin and polytetrafluoroethylene), with an aim to balance corrosion resistance and lubrication effect. However, this type of organic skin film usually has a low cohesive energy. When rapid deep-drawing processing is performed with progressive dies in the field of electrical micro-machines, the organic skin film abrades the surfaces of the dies, which easily leads to interlayer separation of the organic skin film, resulting in black chippings or organic skin film peeling on part surfaces. Not only the appearance of the stamped parts is affected, but also the organic skin film chippings that fall off adhere to the parts or dies, entailing frequent cleaning of the dies and affecting the production efficiency of the stamping production line. At the same time, in order to improve the surface electric conductivity of the parts, a conductive aid such as a strong polar compound, a metal powder or a carbon powder are usually added to the skin film. However, these conductive aids are detrimental to the corrosion resistance of the skin film. That is, they will greatly reduce the corrosion resistance of the skin film, and thus affect the service life of the parts. Meanwhile, along with continuous promulgation of environmental protection directives, chromium-containing galvanized steel sheets have gradually been replaced with environmentally friendly products that do not contain chromium.

At present, chromium-free environmentally friendly products can be roughly classified into an inorganic type and an organic/inorganic composite type according to the type of surface treatment. An inorganic type lubricating skin film is mainly a skin film containing inorganic compounds such as those of silicon, manganese, phosphorus, etc. This type of inorganic skin film has a high cohesive energy, and the inorganic lubricating skin film is less likely to be subjected to interlayer separation or peeling of the skin film due to friction of the dies during a stamping process. Therefore, this type of products can still acquire a good appearance after deep-drawing processing. However, the inorganic type lubricating film cannot significantly improve the corrosion resistance of the galvanized steel sheet, and does not have good surface electric conductivity, so that they cannot be used in areas where relatively high requirements are imposed on grounding safety and electromagnetic characteristics of parts. An organic/inorganic composite type lubricating film is a thin film formed by compounding a resin, a corrosion inhibitor, a silane coupling agent, a silica colloid, and a solid lubricating aid. It exhibits not only excellent lubricity and corrosion resistance, but also good resistances to various chemical media, such as fingerprint resistance, alkali resistance and the like. However, the organic/inorganic composite type lubricating skin film has a relatively high content of the organic resin. The low cohesive energy of the organic resin tends to cause interlayer separation of the organic skin film when rapid deep-drawing processing is performed with progressive dies in the field of electrical micro-machines, which results in black chippings or organic skin film peeling on part surfaces. Not only the appearance of the stamped parts is affected, but also the organic polymer chippings that fall off adhere to the parts or dies, entailing frequent cleaning of the dies and affecting the production efficiency of the stamping production line. At the same time, the organic/inorganic composite type lubricating skin film generally does not have excellent surface electric conductivity, and thus cannot be used in areas where relatively high requirements are imposed on grounding safety and electromagnetic characteristics of parts. Therefore, the chromium-free environmentally friendly products (including inorganic and organic/inorganic composite types) generally used up to now cannot meet the requirements of high-speed deep-drawing characteristics, red rust resistance and surface electric conductivity of materials in the field of electrical micro-machines.

CN 101 376 859 A discloses use of an inorganic treatment agent containing manganese, nickel, phosphate ions and a silane to form a thin transparent inorganic solid film on a surface of a galvanized steel sheet, enabling improvement of stamping formability of the galvanized steel sheet, elimination or alleviation of Zn sticking, pulverization and peeling of the galvanized steel sheet during the stamping forming. Chinese Patent Application Publication No. CN 1177020A (which has been issued as a Chinese Patent) discloses a lubricated steel sheet having a protective film containing silicic acid or a silicate formed on the steel sheet having fine irregularities on its surface, wherein its skin film coverage is about 60%, and the skin film has phosphatability and good lubricity. All of the above patents provide steel sheets with good lubricity, but corrosion resistance thereof is not as good as that of chromium-containing passivated products. Thus, they cannot meet the requirement of red rust resistance of the materials for electrical micro-machines.

CN 101 787 527 A provides a galvanized steel sheet having excellent processability, alkali resistance and solvent resistance, wherein a surface thereof is covered with an organic/inorganic composite protective film comprising an aqueous cationic polyurethane resin, one or more organosilane coupling agents, as well as a corrosion inhibitor and polyoxyethylene particles. The protective film imparts excellent stamping formability, solvent resistance and alkali resistance to the surface of the galvanized steel sheet, and also enables the galvanized steel sheet to have excellent corrosion resistance and coating adhesion. However, in fact, electrical micro-machines have high requirements on surface electric conductivity. The abovementioned organic/inorganic composite protective film does not have excellent surface electric conductivity, and thus cannot be used in areas where relatively high requirements are imposed on grounding safety and electromagnetic characteristics of parts.

CN 101 394 998 A provides a coated steel sheet having excellent bending processability, stamping processability, solvent resistance, chemical resistance, corrosion resistance, and having a good surface appearance and sufficient coating film hardness. However, the steel sheet is a product having a single-layer of thick coating having a film thickness of 2-10 micrometers, and the manufacturing process is a two-step method. First, a chemical conversion skin film containing no chromium is formed, and then a polyester resin is coated. That is, a post-treatment skin film is obtained by two coatings and two bakings. Usually, the second baking requires heating at a steel sheet temperature of 170-250 °C. The coated steel sheet according to this patent is relatively demanding for production equipment, and has no surface electric conductivity, not suitable for use in the field of electrical micro-machines.

CN 105 255 338 A relates to a galvanized steel sheet and a water-based surface treating agent. The surface of a galvanized steel sheet is coated with the surface treating agent in a solidified mode, wherein the surface treating agent includes water-based positive ion polyurethane composite resin, compound organic silane coupling agents containing bis-organic silane coupling agents and mono-organic silane coupling agents, compound lubrication particles containing teflon-surface modification high-density polyethylene particles, oxidized graphene, water-soluble fluorine-containing compounds, water-soluble phosphorous compounds, water-soluble rare earth salt compounds and other components.

CN 105 463 436 A1 discloses an environment-friendly surface treating agent used for a galvanized steel sheet, wherein an aqueous solution of the environment-friendly surface treating agent consists of the following solid components in parts by mass: 30-55 parts of modified enclosed type cationic polyurethane resin (A), 32-60 parts of a silane coupling agent (B) comprising an organic silane coupling agent (B1) with at least one amino functional group of activated hydrogen and an organic silane coupling agent (B2) with at least one epoxy-group functional group in a ratio of B1 to B2 being 0.4-1, 3-15 parts of surface-grafting high-density polyethylene particles or surface-grafting polyamide particles (C), 0.01-0.5 part of a vanadium-containing compound (D) in terms of an element vanadium, 0.5-1.5 parts of a phosphor-containing compound (E) in terms of an element phosphor, 0.1-1 part of a fluorine-containing titanium compound (F) in terms of an element titanium, and 0.01-1 part of a cerium-containing compound (G) in terms of an element cerium.

An inorganic water surface treatment agent for a single-sided electro-galvanized non-chrome surface treatment steel plate, and a single-sided electro-galvanized non-chrome surface treatment steel plate for a fuel tank and a manufacturing method thereof are known from EP 2 957 657 A1. The inorganic water surface treatment agent for a single-sided electro-galvanized non-chrome surface treatment steel plate comprises a metal ion compound containing at least one of Zn2+, Mn2+, Mg2+, Ni2+, A13+ and Ca2+; a vanadium contained compound with at least one of V4+ and V5+; a compound comprising at least one of a phosphoric acid, a pyrophosphoric acid, a metaphosphoric acid, an organic acid and an ammonium salt; a fluoric acid comprising at least one of Zr, Ti, Si, and Ha; a silane coupling agent comprising at least one of a vinyl silane coupling agent, amino silane coupling agent, an epoxy silane coupling agent, and acryloyl silane coupling agent; a silicasol with a grain size of less than 100 nm; and a surface active agent comprising at least one of a carboxylate, a sulfate salt, sulfonate and a phosphate salt. A total solid content of the surface treatment agent is 2wt% to 20wt%. By using the method for manufacturing the a single-sided electro-galvanized non-chrome surface treatment steel plate for a fuel tank, after the surface of the single-sided electro-galvanized steel plate layer is solidified in 70 to 100 °C after the surface is coated by using the foregoing surface treatment agent, and oil coating processing is performed finally, so as to obtain a 10 to600 mg/m² membrane.

### Summary

In view of the above status quo, one object of the present invention is to provide an inorganically surface-treated galvanized steel sheet, a preparation method therefor, and an aqueous inorganic surface treatment agent therefor, wherein the inorganically surface-treated galvanized steel sheet and the aqueous inorganic surface treatment agent therefor are chromium-free and thus environmentally friendly. They can meet the requirements of rapid deep-drawing processing with progressive dies in the field of electrical micro-machines, and at the same time, they impart both excellent red rust resistance and surface electric conductivity to parts, so as to meet the requirements of users in the field of electrical micro-machines on environmental friendliness, surface electric conductivity and red rust resistance of galvanized steel sheets, and on rapid stamping processability.

In order to solve this problem, the present invention provides an inorganically surface-treated galvanized steel sheet as defined in claim 1 and a method of preparing such a inorganically surface-treated galvanized steel sheet as defined in claim 6 as well as an aqueous inorganic surface treatment agent as defined in claim 10. Further improvements are subject to the dependent claims.

The above inorganically surface-treated galvanized steel prepared according to the present invention is chromium free and environmentally friendly, can meet the requirements of rapid deep-drawing processing with progressive dies in the field of electrical micro-machines, and imparts both excellent red rust resistance and surface electric conductivity to parts.

The above inorganically surface-treated galvanized steel prepared according to the method of the disclosure is environmentally friendly and chromium free, can meet the requirements of rapid deep-drawing processing with progressive dies in the field of electrical micro-machines, and imparts both excellent red rust resistance and surface electric conductivity to parts.

In order to ensure a clean surface of a part after rapid deep-drawing with progressive dies and no broken inorganic skin film or zinc powder adhering to the surface of the part, the surface of the part is required to have a "non-stick" characteristic. Accordingly, when it comes to a surface of a steel sheet, only an inorganic skin film is likely to provide such a "non-stick" characteristic. After painstaking research and many attempts, it has been found that, after introduction of a hydrophobic group into a conventional monoorganosilane coupling agent to form a hydrophobic monoorganosilane coupling agent (A), the hydrophobic group in the hydrophobic monoorganosilane coupling agent (A) can migrate to the surface of a skin film during curing of the skin film, forming an extremely thin hydrophobic layer on the surface of the inorganic skin film, thereby reducing the surface polarity and Gibbs free energy of the inorganic skin film, and reducing adhesion of zinc powder, impurities and broken skin film to the inorganic skin film, so as to endow the surface of the inorganic skin film with the "non-stick" characteristic which ensures a clean surface of a part after rapid deep-drawing with progressive dies and no broken inorganic skin film or zinc powder adhering to the surface of the part.

Based on overall consideration, according to the inorganically surface-treated galvanized steel sheet, the method of preparing the same, and the aqueous inorganic surface treatment agent in the present disclosure,
the hydrophobic monoorganosilane coupling agent (A) in the present disclosure should have both a reactive group and a hydrophobic group, and a sum of the number of the reactive group and the number of the hydrophobic group should be 4. In order to ensure that the hydrophobic monoorganosilane coupling agent (A) in the present disclosure have sufficient reactivity to achieve a certain crosslinking density after baking and curing, the number of the reactive group is required to be greater than or equal to two (i.e., may be two or three). Therefore, the number of the hydrophobic group capable of providing the "non-stick" characteristic to the hydrophobic monoorganosilane coupling agent (A) is (4 - the number of the reactive group), indicating that the number of the hydrophobic group in the hydrophobic monoorganosilane coupling agent (A) in the present disclosure may be one or two. The hydrophobic group in the above hydrophobic monoorganosilane coupling agent (A) may be a short-chain hydrocarbyl group such as - CH₃(methyl), -C₂H₅(ethyl), -C₃H₇(propyl) or -C₆H₅(phenyl); or may be a fluorine-containing hydrophobic group such as -CF₃ (perfluoromethyl), -C₂F₅ (perfluoroethyl), -C₃F₇ (perfluoropropyl), -C₅F₁₁ (perfluoropentyl), -C₇F₁5 (perfluoroheptyl) or -C₉F₁₉ (perfluorononyl). The hydrophobic group in the hydrophobic monoorganosilane coupling agent (A) in the present disclosure may be any one or two of the above groups.

In summary, according to the inorganically surface-treated galvanized steel sheet, the method of preparing the same, and the aqueous inorganic surface treatment agent of the present invention,
the hydrophobic monoorganosilane coupling agent (A) in the present disclosure should have both a reactive group (two or three) and a hydrophobic group (one or two) in its structure, and a sum of the number of the reactive group and the number of the hydrophobic group is 4. For example, those that may be exemplified include a trimethoxymethylsilane coupling agent, a triethoxymethylsilane coupling agent, a tripropoxymethylsilane coupling agent, a trimethoxyethylsilane coupling agent, a triethoxyethylsilane coupling agent, a tripropoxyethylsilane coupling agent, a trimethoxypropylsilane coupling agent, a triethoxypropylsilane coupling agent, a tripropoxypropylsilane coupling agent, a 3-aminopropyl-ethoxy-methylsilane coupling agent, a N-(2-aminoethyl)-aminopropylmethyldimethoxysilane coupling agent, a 1H, 1H, 2H, 2H-perfluorodecyltrimethoxysilane coupling agent, a 1H, 1H, 2H, 2H-per-fluorodecyltriethoxysilane coupling agent, a 1H, 1H, 2H, 2H-perfluorooctyltrimethoxysilane coupling agent, a 1H, 1H, 2H, 2H-perfluorooctyltriethoxysilane coupling agent, methylphenyldiethoxysilane, diphenyldiethoxysilane, fluoromethyltrimethoxysilane, fluoromethyltriethoxysilane, fluoromethylethoxydimethoxysilane, fluoroethyltrimethoxysilane, fluoroethyltriethoxysilane, 3-fluoropropylmethyldimethoxysilane, 3-fluoropropylmethyldiethoxysilane, 3-fluoropropyltriethoxysilane, etc. Any one or two or more of the above silane coupling agents may be used as the hydrophobic monoorganosilane coupling agent (A).

The hydrophobic monoorganosilane coupling agent (A) in the present disclosure is 40-60 parts by weight of the inorganic skin film. If it is less than 40 parts, the corrosion resistance and "non-stick" characteristic of the inorganic skin film will be poor, wherein poor corrosion resistance of the inorganic skin film may affect the red rust resistance of stamped parts; and poor "non-stick" characteristic may lead to adhesion of a lot of impurities to the part surface after stamping, affecting the appearance of the stamped parts. If it is more than 60 parts, the ductility of the inorganic skin film will be deteriorated, and the inorganic skin film is liable to crack and peel off during a forming process, resulting in decreased stamping formability of the skin film.

According to the inorganically surface-treated galvanized steel sheet, the method of preparing the same, and the aqueous inorganic surface treatment agent in the present disclosure,
the systematic crosslinking agent (B) used in the present disclosure comprises a large number of reactive groups which can be chemically bonded to a metal substrate and the other components in the inorganic skin film. This can not only improve adhesion between the inorganic skin film and the metal substrate, but also enhance the crosslinking density of the inorganic skin film to achieve the purpose of enhancing the corrosion resistance and stamping formability of the inorganic skin film, so that stamped parts have excellent red rust resistance and surface appearance.

According to the inorganically surface-trcatcd galvanized steel sheet, the method of preparing the same, and the aqueous inorganic surface treatment agent in the present disclosure,
the systematic crosslinking agent (B) in the present disclosure may be one or more of an orthosilicate, a titanate or a diorganosilane coupling agent having a bridging structure; the orthosilicate comprises 4 reactive groups, wherein the reactive group may be any one of a methoxy group, an ethoxy group, a propoxy group or a n-butoxy group; the titanate comprises four reactive groups, wherein the reactive group may be one or more of an isopropyl ester group, a phosphoryloxy group, a benzenesulfonyloxy group or a n-butyl ester group; and the diorganosilane coupling agent means that two silane structures exist in the same molecular structure, wherein one molecule comprises 6 reactive groups, and the number of reactive groups is larger than that of a conventional monoorganosilane coupling agent. The diorganosilane coupling agent in the present disclosure comprises a bridging structure consisting of 2-4 methylene groups, amino groups or 2-4 mercapto groups, wherein the reactive group of the diorganosilane coupling agent may be any one of a methoxy group, an ethoxy group or a propoxy group.

According to the inorganically surface-treated galvanized steel sheet, the method of preparing the same, and the aqueous inorganic surface treatment agent in the present disclosure,
the orthosilicate used in the systematic crosslinking agent (B) in the present disclosure may be one or more of methyl orthosilicate, ethyl orthosilicate, propyl orthosilicate, butyl orthosilicate or isopropyl orthosilicate; the titanate used in the systematic crosslinking agent (B) in the present disclosure may be one or more of tetraisopropyl orthotitanate, isopropyl tris(dioctylphosphoryloxy) titanate, isopropyl trioleyl titanate, tetraisopropyl bis(dioctylphosphate) titanate, bis(dioctyloxypyrophosphate) ethylene titanate, isopropyl tris(do-decylbenzenesulfonyl) titanate, tetra-tert-butyl orthotitanate or diisopropyl bis(triethanolamine) titanate; and the diorganosilane coupling agent used in the systematic crosslinking agent (B) in the present disclosure may be one or more of 1,2-bistrimethoxysilylethane, 1,2-bisethylmethoxysilylethane, bis-(y-triethoxysilylpropyl) tetrasulfide, bis-[γ-(triethoxysilyl)propyl] disulfide, bis-(y-trimethoxysilylpropyl) amine. The systematic crosslinking agent (B) used in the present disclosure may be any one or more of the above-mentioned orthosilicates, titanates and diorganosilane coupling agents.

According to the inorganically surface-treated galvanized steel sheet, the method of preparing the same, and the aqueous inorganic surface treatment agent in the present disclosure,
the systematic crosslinking agent (B) in the present disclosure is 10-30 parts by weight of the inorganic skin film. If it is less than 10 parts, the crosslinking density of the inorganic skin film will be lowered greatly, thereby affecting the corrosion resistance of the inorganic skin film, and ultimately, the red rust resistance of stamped parts will be poor. If it is higher than 30 parts, because compatibility of a selected systematic crosslinking agent with water is not very good, the systematic crosslinking agent in a high amount will affect stability of the aqueous inorganic surface treatment agent, which will result in obvious stratification of the treatment agent after standing for a long time, leading to large decrease in the overall performance of the aqueous inorganic surface treatment agent.

According to the inorganically surface-treated galvanized steel sheet, the method of preparing the same, and the aqueous inorganic surface treatment agent in the present disclosure,
the water-soluble nanosol (C) used in the present disclosure is preferably a water-soluble colloid having a particle diameter of 5 - 50 nm, and it may be a type of aqueous inorganic oxide or metal oxide sol. Specifically, it may be one or more of a silica sol, an aqueous titania sol, an aqueous zirconia sol or an aqueous alumina sol. The crosslinking density of the inorganic skin film can be further increased by a large number of reactive groups in the aqueous nanosol, thereby enhancing the corrosion resistance of the inorganic skin film. At the same time, fine particles formed by baking and curing the aqueous nanosol have high hardness, which can effectively improve scratch resistance of the inorganic skin film and avoid surface scratches on stamped parts.

According to the inorganically surface-treated galvanized steel sheet, the method of preparing the same, and the aqueous inorganic surface treatment agent in the present disclosure,
the water-soluble nanosol (C) used in the present disclosure may be an aqueous silica sol, such as SNOWTEX-40, SNOWTEX-50, SNOWTEX-C, SNOWTEX-N, SNOWTEX-O, SNOWTEX-OL, SNOWTEX-ZL and SNOWTEX-UP from Nissan Chemical; LUDOX-AM, LUDOX-AS, LUDOX-CL, LUDOX-DF, LUDOX-HS, LUDOX-LS, LUDOX-SK, LUDOX-SM, LUDOX-TM and LUDOX-TMA from Grace, the USA; ADELITE AT-20N or ADELITE AT-20A from Asahi Denka, Japan; the water-soluble nanosol (C) used in the present disclosure may also be an aqueous titanium dioxide sol, such as MTI-2080 from Shenzhen Yoshida Chemical; EFUT- GY01, EFUT-GY02, EFUT-GY03 from Shanghai Yifu, etc; the water-soluble nanosol (C) used in the present disclosure may also be an aqueous zirconia sol, such as VK-RJ80 from Xuancheng Jingrui, GT-360 from Yizhen Technology, UG03W, UG-R10W and UR-R30W from Suzhou Yougao, etc; and the water-soluble nanosol (C) used in the present disclosure may be an aqueous alumina sol, such as SH-33 from Qingdao Shankehaitai, LA-20 from Ji'nan Fujing, EFUAL-Y10C, EFUAL-Y10S, EFUAL-Y20C, EFUAL-Y20S, EFUAL-Y30C and EFUAL-Y30S from Shanghai Yifu, etc. The aqueous nanosol (C) used in the present disclosure may be any one or more of the above aqueous silica sols, aqueous titania sols, aqueous zirconia sols or aqueous alumina sols.

According to the inorganically surface-treated galvanized steel sheet, the method of preparing the same, and the aqueous inorganic surface treatment agent in the present disclosure,
the aqueous nanosol (C) in the present disclosure is 5-15 parts by weight of the inorganic skin film. If it is less than 5 parts, the surface hardness of the inorganic skin film will be lowered greatly, thereby affecting the scratch resistance of the inorganic skin film, such that the inorganic skin film will be easily damaged during a stamping forming process. If it is more than 15 parts, there will be too many nanoparticles in the inorganic skin film, and thus the ductility of the skin film will be deteriorated, resulting in decreased stamping formability of the skin film.

According to the inorganically surface-treated galvanized steel sheet, the method of preparing the same, and the aqueous inorganic surface treatment agent in the present disclosure,
the surface-modified high-density polyethylene particles (D) used in the present disclosure are commercially available solid lubricating particles. This kind of lubricating aid is characterized by low surface energy, high lubricity and high surface hardness. It can form a hard lubricating layer on the surface of the inorganic skin film, which can not only improve scratch resistance of the inorganic skin film, but also enhance surface smoothness of the inorganic skin film, thereby achieving the purpose of improving the stamping formability of the inorganic skin film, so that the inorganic skin film can meet the requirements of rapid deep-drawing processing with progressive dies in the field of electrical micro-machines. In the field of electrical micro-machines, progressive die stamping usually exceeds 10 passes, and each pass of stamping causes frictional wear to the inorganic skin film in the present disclosure. To ensure the appearance and corrosion resistance of stamped parts, the inorganic skin film in the present disclosure is required to have strong scratch resistance and be able to ensure integrity and excellent appearance of the skin film during the multi-pass stamping process. After painstaking research and attempts, it has been found that if it is necessary to ensure that the inorganic skin film in the present disclosure should have the above properties, it is necessary to precisely control the distribution of the composite lubricating particles used in the present disclosure in the inorganic skin film, so that a small amount of the solid lubricating particles can gather in the surface of the inorganic skin film, and the solid lubricating particles can also be dispersed uniformly inside the inorganic skin film. Thus, the inorganic skin film exhibits excellent scratch resistance across the entire thickness, thereby ensuring that the inorganic skin film can meet the requirements of multi-pass progressive die stamping.

According to the inorganically surface-treated galvanized steel sheet, the method of preparing the same, and the aqueous inorganic surface treatment agent in the present disclosure,
the surface-modified high-density polyethylene particles (D) used in the present disclosure are solid lubricating particles having a reactive group grafted on a particle surface. Specifically, the reactive group may be one or more of an amino group, a hydroxyl group, a carboxyl group, an epoxy group or a urethane group, wherein the hydroxyl group and the carboxyl group can be obtained by immersing the high-density polyethylene particles in a strong oxidative solution; the amino group and the urethane group can be obtained by grafting ethylenediamine, hexamethylenediamine or ethyl urethane to the surface of the high-density polyethylene particles; and the epoxy group can be obtained by grafting glycidyl methacrylate or allyl glycidyl ether to the surface of the high-density polyethylene particles. The above reactive groups can react with the organosilane coupling agent in the treatment solution to form a covalent bond, which can not only enhance the bonding strength between the high-density polyethylene particles and the inorganic skin film, but also confine the high-density polyethylene particles, thereby ensuring that the high-density polyethylene particles can be uniformly dispersed in the inorganic skin film, provide excellent anti-wear property across the entire thickness of the inorganic skin film, and improve the stamping processability and scratch resistance of the inorganic skin film. At the same time, the chemical bonding between the high-density polyethylene particles and the skin film can delay penetration of a corrosive medium along the surface of the high-density polyethylene particles into the skin film, and alleviate the negative influence of the addition of the high-density polyethylene particles on the corrosion resistance of the inorganic skin film.

According to the inorganically surface-treated galvanized steel sheet, the method of preparing the same, and the aqueous inorganic surface treatment agent in the present disclosure,
the surface-modified high-density polyethylene particles (D) used in the present disclosure have a particle diameter in the range of 0.1-0.5 µm. If the particle diameter is less than 0.1 µm, the surface-modified high-density polyethylene particles (D) in the inorganic skin film will not have the effect of enhancing the scratch resistance of the inorganic skin film. If the particle diameter is higher than 0.5 µm, the surface-modified high-density polyethylene particles (D) will be too large, and most of the particles will be exposed on the surface of the skin film. When subjected to stamping friction, large particles will be easily detached. As a result, the stamping processability of the skin film will be lowered drastically.

According to the inorganically surface-treated galvanized steel sheet, the method of preparing the same, and the aqueous inorganic surface treatment agent in the present disclosure,
the surface-modified high-density polyethylene particles (D) used in the present disclosure are 10-25 parts by weight of the inorganic skin film. If the content is less than 10 parts, the surface of the inorganic skin film will not have sufficient lubricity and scratch resistance. If the content is more than 25 parts, too many surface-modified high-density polyethylene particles (D) will be present in the inorganic skin film, and the corrosive medium may penetrate into the inorganic skin film along the interface of the surface-modified high-density polyethylene particles (D), thereby reducing the corrosion resistance of the inorganic skin film.

According to the inorganically surface-treated galvanized steel sheet, the method of preparing the same, and the aqueous inorganic surface treatment agent in the present disclosure,
the inorganically surface-treated galvanized steel sheet of the present disclosure needs to have good surface electric conductivity, and be able to discharge the static electricity generated during the actual operation of a stamped and formed part through the surface thereof, thereby preventing accumulation of a large amount of electrostatic charge on the surface of the part. Otherwise, the safety and electromagnetic characteristics of the part will be affected, and thus normal use of the part will be affected. After painstaking research and attempts, it has been found that advantage of the excellent electric conductivity of a graphene sheet may be taken to significantly improve the surface electric conductivity of the inorganically surface-treated galvanized steel sheet in the present disclosure by adding an appropriate amount of graphene sheets to the inorganic skin film of the galvanized steel sheet.

Further, the abovementioned graphene sheets need to be stably present in the aqueous inorganic surface treatment agent for a long period of time without agglomeration, precipitation, or segregation. However, due to the large van der Waals force between the graphene sheets, the graphene sheets are particularly prone to agglomeration, and cannot be easily dispersed in the aqueous inorganic surface treatment agent uniformly. Therefore, it is necessary to modify the surface of the graphene sheets. By introducing other substances to destroy the surface van der Waals force, the graphene sheets are separated from each other, so that they can be stably present in the aqueous inorganic surface treatment agent for a long period of time. In order for the graphene sheets to be stably present in the aqueous inorganic surface treatment agent of the present disclosure for a long period of time, the substance used to modify the graphene surface needs to be further defined. In view of the fact that the main components of the aqueous inorganic surface treatment agent of the present disclosure are mostly silicon-containing substances, such as a hydrophobic monoorganosilane coupling agent (A), a systematic crosslinking agent (B) and a water-soluble nanosol (C), etc, the present disclosure utilizes an orthosilicate as a modifying substance and propanol as a solvent to modify the surface of the graphene sheets with an aim to further improve dispersibility of the graphene sheets, and improve compatibility between the graphene sheets and the aqueous inorganic surface treatment agent.

According to the inorganically surface-treated galvanized steel sheet, the method of preparing the same, and the aqueous inorganic surface treatment agent in the present disclosure,
the graphene sheet used in the present disclosure has a layered structure, and may be monolayered or multilayered. When the graphene is multilayered, the number of sheet layers is preferably 5 or less (a sheet layer has a thickness of between 0.35 and 1.75 nm). Further, the graphene sheet used in the present disclosure has a sheet diameter of 2-5 µm and a graphene aspect ratio of 1100-14000. By controlling the number of graphene oxide layers to 5 or less and the sheet diameter to 2-5 µm, graphene can maintain excellent electric conductivity and easily form a conductive network in the inorganic skin film, thereby improving the surface electric conductivity of the inorganic skin film.

The surface of the graphene sheet used in the present disclosure is modified with an orthosilicate, and a method known to date for preparation of a surface-modified graphene sheet can be used. For example, first, a graphite oxide may be immersed in a strong oxidative solution (such as a mixed solution of concentrated sulfuric acid/potassium permanganate, a mixed solution of concentrated sulfuric acid/concentrated nitric acid) at 70-80 °C and ultrasonically dispersed for 1 hour, and then filtered and washed with a large amount of deionized water to neutral to obtain a graphene oxide sheet; further, the graphene oxide sheet is mixed with an orthosilicate and propanol under agitation at 100 °C for 24 h, and then filtered to obtain an orthosilicate-modified graphene oxide; secondly, the orthosilicate-modified graphene oxide is diluted with propanol to a mass fraction of 1-5%.

The orthosilicate used for the orthosilicate-modified graphene oxide used in the present disclosure may be one or more of methyl orthosilicate, ethyl orthosilicate, propyl orthosilicate or butyl orthosilicate. In the orthosilicate-modified graphene oxide according to the disclosure, the ratio of the number of carbon atoms to the number of oxygen atoms is <3, and the silicon element has a content of 5-12%.

The orthosilicate-modified graphene oxide according to the present disclosure comprises a surface-grafted orthosilicate, which can not only increase the dispersion stability coefficient of the graphene oxide in the aqueous inorganic surface treatment agent system and prevent agglomeration or precipitation thereof, but also promote chemical bonding reactions of the graphene oxide with the hydrophobic monoorganosilane coupling agent (A), the systematic crosslinking agent (B) and the water-soluble nanosol (C) in the system, so that the graphene oxide is more likely to form a conductive network in the inorganic skin film, and enhance the effect of the graphene oxide in increasing the surface electric conductivity of the inorganic skin film. Further, the graphene oxide having a layered structure is uniformly dispersed inside the inorganic skin film. When a corrosive medium attempts to penetrate into the inorganic skin film, the sheet layers of the graphene oxide can extend the permeation path of the corrosive medium, thereby providing excellent physical protection and thus greatly improving the corrosion resistance of the skin film. At the same time, the atoms in the graphene oxide sheet are linked by carbon-carbon covalent bond. Hence, the graphene oxide sheet has excellent mechanical properties, and has good resistance to wear and damage caused by external objects. Therefore, it has a function in improving the scratch resistance of the inorganic skin film.

According to the inorganically surface-treated galvanized steel sheet, the method of preparing the same, and the aqueous inorganic surface treatment agent in the present disclosure,
the orthosilicate-modified graphene oxide used in the present disclosure is 0.05-0.5 parts by weight of the inorganic skin film based on graphene oxide. If the content is less than 0.05 parts, that is, when too little graphene oxide is used, the graphene oxide will have no obvious effect in improving the surface electric conductivity of the inorganic skin film. If the content is higher than 0.5 parts, that is, when too much graphene oxide is used, the inorganic skin film will become dark under the influence of the graphene oxide, and its appearance will be affected. At the same time, when too much graphene oxide is used, it's prone to agglomeration, which will decrease the surface quality of the inorganic skin film.

The fluorine-containing compound used in the present disclosure is water-soluble, and may be a fluorine-containing metal salt or a fluorine-containing acid. For example, the fluorine-containing compound may be one or more of sodium fluoride, ammonium fluorotitanate, sodium fluorosilicate, hexafluorotitanic acid, and fluorosilicic acid. The mass fraction of the fluorine-containing compound in the inorganic skin film is 1-4 parts based on the fluorine element in the fluorine-containing compound. If the mass fraction of the fluorine element is less than 1 part, that is, when too little fluorine-containing compound is used, the corrosion resistance of the inorganic skin film may decrease. If the mass fraction of the fluorine element is more than 4 parts, that is, when too much fluorine-containing compound is used, the aqueous inorganic surface treatment agent may become less stable.

The phosphorus-containing compound used in the present disclosure is water-soluble, and may be a phosphate salt or a phosphorus-containing acid. For example, the phosphorus-containing compound may be one or more of orthophosphoric acid, pyrophosphoric acid, triphosphoric acid, trimetaphosphoric acid, ammonium phosphate, aluminum triphosphate and ammonium polyphosphate. The mass fraction of the phosphorus-containing compound in the inorganic skin film is 0.5-4 parts based on the phosphorus element in the phosphorus-containing compound. If the mass fraction of the phosphorus element is less than 0.5 parts, that is, when too little phosphorus-containing compound is used, the addition thereof will have no effect, and the corrosion resistance of the inorganic skin film may decrease. If the mass fraction of the phosphorus element is more than 4 parts, that is, when too much phosphorus-containing compound is used, the inorganic skin film may become less adhesive.

The metal salt compound used in the present disclosure is a water-soluble salt, and may be one or more of a titanium salt, a cerium salt, a lanthanum salt, a molybdenum salt, a tungsten salt, a cobalt salt, and a zirconium salt. For example, the titanium salt may be one or more of ammonium fluorotitanate, hexafluorotitanic acid, titanium orthosulfate, titanium oxysulfate or titanium chloride; the cerium salt may be cerium nitrate, cerium sulfate, or may be a fluorine-containing cerium salt, or may be one or more of composite salts of cerium and ammonium; the lanthanum salt may be one or more of lanthanum chloride, lanthanum sulfate, and lanthanum nitrate; the molybdenum salt may be one or more of ammonium molybdate, magnesium molybdate or sodium molybdate; the tungsten salt may be one or more of ammonium tungstate, magnesium tungstate, ammonium paratungstate or ammonium metatungstate; the cobalt salt may be an inorganic cobalt salt such as cobalt nitrate, cobalt sulfate or cobalt chloride, or one or more of cobalt naphthenate, cobalt oxalate or cobalt stearate; and the zirconium salt may be one or more of potassium fluorozirconate, zirconium nitrate, and zirconium sulfate. The metal salt compound can react with a zinc coating on a surface of the galvanized steel sheet and hydroxyl groups of the other components in the aqueous inorganic surface treatment agent to form metallic bonds having a high bond energy, thereby forming a thin layer of metal salt conversion film having a dense structure on the surface of the zinc coating. The metal salt conversion film physically prevents direct contact between the steel sheet and a corrosive medium, reduces the possibility of corrosion of the steel sheet, and thus significantly improves the ability of the steel sheet to resist expansion of under-film corrosion. The mass fraction of the metal salt compound in the skin film is 0.1-2.5 parts based on the metal element. If the mass fraction of the rare earth elements is less than 0.1 part, that is, when too little metal salt compound is used, the addition thereof will have no effect, and the corrosion resistance and adhesion of the inorganic skin film may be lowered. If the mass fraction of the rare earth elements is more than 2.5 parts, that is, when too much metal salt-containing compound is contained, the aqueous inorganic surface treatment agent will become less stable, and the quality of the inorganically surface-treated galvanized steel sheet may be affected.

According to the inorganically surface-treated galvanized steel sheet, the method of preparing the same, and the aqueous inorganic surface treatment agent in the present disclosure,
the disclosure provides a method of manufacturing an environmentally-friendly, inorganically surface-treated galvanized steel sheet which can meet the requirements of rapid deep-drawing processing with progressive dies in the field of electrical micro-machines and imparts excellent red rust resistance and surface electric conductivity to parts. The steel sheet is dried at a temperature of 60-120°C. If the temperature is lower than 60°C, crosslinking reactions in the inorganic skin film will not proceed sufficiently, which may lead to degradation of various properties of the inorganic skin film. If the temperature is higher than 120 °C, the properties of some components in the aqueous inorganic surface treatment agent may change, and the film-forming effect may be affected.

According to the inorganically surface-treated galvanized steel sheet, the method of preparing the same, and the aqueous inorganic surface treatment agent in the present disclosure,
the aqueous inorganic surface treatment agent in the disclosure is applied on a surface of a galvanized steel sheet, and a dry film thickness thereof is between 0.3 and 1 micrometer. If the thickness is less than 0.3 micrometers, the inorganic skin film will be rather thin, which may lead to degradation of the stamping processability and red rust resistance of the inorganic skin film. If the thickness of the inorganic skin film exceeds 1 micrometer, surface treatment cost per unit area will be increased.

The method of heating and drying the aqueous inorganic surface treatment agent applied on the surface of the galvanized steel sheet is not particularly limited, and may be hot air heating, induction heating, infrared heating or the like. The size, shape, and the like of the galvanized steel sheet are not particularly limited in the present disclosure. The galvanized steel sheet useful in the present disclosure may be a steel sheet electroplated with pure zinc, a hot-dip pure zinc coated steel sheet, a hot-dip zinc-aluminum coated steel sheet, or an alloyed hot-dip galvanized steel sheet.

In an open environment, the aqueous inorganic surface treatment agent of the present disclosure can form an inorganic skin film on a surface of a galvanized steel sheet after coating and low temperature rapid curing (less than 100 °C). The galvanized steel sheet coated with the inorganic skin film needs to meet the requirements of rapid deep-drawing processing with progressive dies, such as no die blocking, part appearance, dimensional precision and surface cleanness, and also has excellent red rust resistance of a part, surface electric conductivity and non-sticking of the skin film. Specifically, stamping without die blocking requires that a part can be detached from a die naturally under gravity after rapid stamping (the stamping mold will be damaged if the stamped part is stuck to a die at a certain station of a progressive die stamping process and cannot be detached naturally), so that the naturally detached part can automatically arrive at the next stamping station under the guidance of tapping. As the appearance of a stamped part is concerned, the surface of the stamped part is required to be free of surface defects such as blackening, brightening, scratches, black spots or streaks due to stamping. At the same time, the surface of the stamped part is clean, with no broken skin film or zinc powder adhered to the surface. Red rust resistance of a part is mainly utilized to evaluate the corrosion resistance of the part by observing appearance of red rust on the surface of the stamped part. Excellent red rust resistance ensures that the material can be used nakedly with no need of post-coating. Surface electric conductivity mainly means that the surface of a galvanized steel sheet coated with the inorganic skin film should have certain electric conductivity, thereby ensuring grounding safety and electromagnetic characteristics of the formed part.

The disclosure has the following beneficial effects in comparison with the prior art:
1) The present disclosure uses a hydrophobic monoorganosilane coupling agent having both a hydrophobic group and a reactive group as a main film-forming component, such that an inorganic skin film further possesses hydrophobicity and low surface energy properties in addition to excellent red rust resistance. Hence, a "non-stick" characteristic of the inorganic skin film is achieved, thereby enabling a part to maintain excellent surface cleanness after rapid deep-drawing processing with progressive dies.
2) The disclosure utilizes a systematic crosslinking agent with a plurality of reactive groups and a water-soluble nanosol, thereby further enhancing the crosslinking degree of the inorganic skin film in three dimensions, so that the red rust resistance, hardness and scratch resistance of the inorganic skin film are increased greatly.
3)The reactive group in the surface-modified high-density polyethylene particles of the present disclosure can react with various main components in a treatment solution to form covalent bond linkages, which can not only increase the bonding strength between the high-density polyethylene particles and the inorganic skin film, but also confine the high-density polyethylene particles to ensure that the high-density polyethylene particles can be uniformly dispersed in the inorganic skin film, provide excellent anti-wear property across the entire thickness of the inorganic skin film, and improve the stamping processability and scratch resistance of the inorganic skin film.
4) The disclosure uses a graphene oxide with a layered structure comprising 5 or less layers, and grafts an orthosilicate on a surface thereof, so as to improve dispersion stability of the graphene oxide in the aqueous inorganic surface treatment agent system, and enhance chemical bonding reactions of the graphene oxide with the hydrophobic monoorganosilane coupling agent (A), the systematic crosslinking agent (B) and the water-soluble nanosol (C) in the aqueous inorganic surface treatment system. Therefore, the graphene oxide is more likely to form a conductive network in the inorganic skin film, and enhance the effect of the graphene oxide in increasing the surface electric conductivity of the inorganic skin film.
5) The aqueous inorganic surface treatment agent of the present disclosure is chromium-free. So, it is an environmentally-friendly surface treatment agent. After surface treatment of a galvanized steel sheet with the aqueous inorganic surface treatment agent, the galvanized steel sheet can meet the requirements of rapid deep-drawing processing with progressive dies in the field of electrical micro-machines, and impart both excellent red rust resistance and surface electric conductivity to parts.

### Detailed Description

The disclosure will be further illustrated with reference to the following specific Examples. However, the scope of the disclosure is not limited to these Examples. In the following Examples and Comparative Examples, the galvanizing materials, surface cleaning processes and aqueous inorganic surface treatment agents that are used are described as follows.

### Examples

### (1) Substrates

The types of substrates used are shown in Table 1. For substrates to be coated with inorganic skin films, mild steel having a thickness of 0.5 mm was used. The substrates in Table 1 were spray cleaned using an aqueous solution of an alkaline degreaser having a mass fraction of 2% (trade name: FC-364S, manufactured by Shanghai Parkerizing). Aqueous solution temperature: 50 °C; spray time: 60 seconds. Then, they were washed with industrial pure water to remove the alkaline component remaining on the surface, and dried with a blower for use.

**Table 1: Substrates**

| No. | Sample Type | Note |
|---|---|---|
| S1 | Steel sheet electroplated with pure zinc | Coating weight 20/20 g/m² |
| S2 | Hot-dip pure zinc coated steel sheet | Coating weight 60/60 g/m² |
| S3 | Hot-dip zinc-aluminum coated steel sheet | Al in the coating: 5wt%; coating weight 60/60 g/m² |
| S4 | Alloyed hot-dip galvanized steel sheet | Fe in the coating: 10wt%; coating weight 45/45 g/m² |

### (2) Aqueous inorganic surface treatment agents

An aqueous inorganic surface treatment agent for forming an inorganic skin film was formulated by using a hydrophobic monoorganosilane coupling agent (Table 2), a systematic crosslinking agent (Table 3), a water-soluble nanosol (Table 4), and surface-modified high-density polyethylene particles (Table 5), an orthosilicate-modified graphene oxide (Table 6), a water-soluble fluorine-containing compound (Table 7), a water-soluble phosphorus-containing compound (Table 8) and a water-soluble metal salt compound (Table 9) in blending amounts shown in Table 10, and samples were prepared in accordance with the sample types and sample preparation conditions shown in Table 10.

**Table 2: Monoorganosilane coupling agents**

| No. | Monoorganosilane coupling agent |
|---|---|
| A1 | Trimethoxymethylsilane coupling agent |
| A2 | Triethoxymethylsilane coupling agent |
| A3 | Tripropoxymethylsilane coupling agent |
| A4 | Trimethoxyethylsilane coupling agent |
| A5 | Triethoxyethylsilane coupling agent |
| A6 | Trimethoxypropylsilane coupling agent |
| A7 | Triethoxypropylsilane coupling agent |
| A8 | 3-aminopropyl-ethoxy-methylsilane coupling agent |
| A9 | N-(2-aminoethyl)-aminopropylmethyldimethoxysilane coupling |
| A10 | 1H,1H,2H,2H-perfluorodecyltrimethoxysilane coupling agent |
| A11 | 1H,1H,2H,2H-perfluorodecyltriethoxysilane coupling agent |
| A12 | 1H,1H,2H,2H-perfluorooctyltrimethoxysilane coupling agent |
| A13 | 1H,1H,2H,2H-perfluorooctyltriethoxysilane coupling agent |
| A14 | Methylphenyldiethoxysilane |
| A15 | Fluoromethylethoxydimethoxysilane |
| A16 | Fluoroethyltriethoxysilane |
| A17 | 3 -fluoropropylmethyldiethoxysilane |

**Table 3: Systematic crosslinking agents**

| No. | Systematic crosslinking agent |
|---|---|
| B1 | Ethyl orthosilicate |
| B2 | Propyl orthosilicate |
| B3 | Butyl orthosilicate |
| B4 | Tetraisopropyl orthotitanate |
| B5 | Isopropyl tris(dioctylphosphoryloxy) titanate |
| B6 | Isopropyltris(dodecylbenzenesulfonyl) titanate |
| B7 | 1,2-bisethylmethoxysilylethane |
| B8 | Bis-(γ-triethoxysilylpropyl)tetrasulfide |
| B9 | Bis-(γ-trimethoxysilylpropyl)amine |

**Table 4: Water-soluble nanosols**

| No. | Water-soluble nanosol |
|---|---|
| C1 | Water-soluble nanosilica sol SNOWTEX-O |
| C2 | Water-soluble nanosilica sol SNOWTEX-40 |
| C3 | Water-soluble nanosilica sol LUDOX-AS |
| C4 | Water-soluble nanosilica sol ADELITE AT-20N |
| C5 | Water-soluble titanium dioxide sol EFUT-GY01 |
| C6 | Water-soluble zirconia sol UG-R10W |
| C7 | Water-soluble zirconia sol VK-RJ80 |
| C8 | Water-soluble alumina sol EFUAL-Y10C |

**Table 5: Surface-modified high density polyethylene particles**

| No. | Surface-modified high density polyethylene particles |
|---|---|
| D1 | Amino-surface-modified high-density polyethylene particles: particle size 0.1 µm |
| D2 | Amino-surface-modified high-density polyethylene particles: particle size 0.3 µm |
| D3 | Amino-surface-modified high-density polyethylene particles: particle size 0.5 µm |
| D4 | Carboxyl-surface-modified high-density polyethylene particles: particle size 0.1 µm |
| D5 | Carboxyl-surface-modified high-density polyethylene particles: particle size 0.3 µm |
| D6 | Carboxyl-surface-modified high-density polyethylene particles: particle size 0.5 µm |

**Table 6: Orthosilicate-modified graphene oxides**

| No. | Orthosilicate-modified graphene oxide |
|---|---|
| E1 | Methyl orthosilicate-modified graphene oxide: 1-3 layers, sheet diameter 2-3 microns |
| E2 | Methyl orthosilicate-modified graphene oxide: 4-5 layers, sheet diameter 2-5 microns |
| E3 | Ethyl orthosilicate-modified graphene oxide: 1-3 layers, sheet diameter 2-3 microns |
| E4 | Ethyl orthosilicate-modified graphene oxide: 4-5 layers, sheet diameter 2-5 microns |
| E5 | Propyl orthosilicate-modified graphene oxide: 1-3 layers, sheet diameter 2-3 microns |
| E6 | Propyl orthosilicate-modified graphene oxide: 4-5 layers, sheet diameter 2-5 microns |

**Table 7: Water-soluble fluorine-containing compounds**

| No. | Water-soluble fluorine-containing compound |
|---|---|
| F1 | Sodium fluoride |
| F2 | Ammonium fluorotitanate |
| F3 | Sodium fluorosilicate |
| F4 | Hexafluorotitanic acid |

**Table 8: Water-soluble phosphorus-containing compounds**

| No. | Water-soluble phosphorus-containing compound |
|---|---|
| G1 | Orthophosphoric acid |
| G2 | Triphosphoric acid |
| G3 | Ammonium phosphate |
| G4 | Polyammonium phosphate |

**Table 9: Water-soluble metal salts**

| No. | Water-soluble metal salt |
|---|---|
| H1 | Titanium oxysulfate |
| H2 | Cerium nitrate |
| H3 | Lanthanum nitrate |
| H4 | Ammonium molybdate |
| H5 | Ammonium paratungstate |
| H6 | Cobalt nitrate |
| H7 | Potassium fluorozirconate |

**Table 10: Aqueous inorganic surface treatment agents**

| No. | Substrate | Hydrophobic monoorganosilane coupling agent (A) | | Systematic cross- linking agent (B) | | Water-soluble na nosol (C) | | Surface-modified high density polyethylene particles (D) | | Orthosilicate-modified graphene oxide (E) | | Water-soluble fluorine-containing compound (F) | | Water-soluble phosphorus-containing compound (G) | | Water-soluble metal salt (H) | | Coating weight g/m² | PMT °C |
|---|---|---|---|---|---|---|---|---|---|---|---|---|---|---|---|---|---|---|---|
| | | Type | Parts by weight | Type | Parts by weight | Type | Parts by weight | Type | Parts by weight | Type | Parts by weight | Type | Parts by weight | Type | Parts by weight | Type | Parts by weight | | |
| Ex. 1 | S1 | A1 | 50 | B1 | 15 | C1 | 7 | D1 | 15 | E2 | 0.05 | F1 | 1.5 | G1 | 1.5 | H1 | 1.2 | 0.6 | 100°C |
| Ex. 2 | S1 | A2 | 50 | B1 | 16 | C1 | 8 | D1 | 15 | E2 | 0.1 | F1 | 1.5 | G1 | 1.7 | H1 | 1.2 | 0.6 | 100°C |
| Ex. 3 | S1 | A3 | 50 | B1 | 17 | C1 | 9 | D1 | 15 | E2 | 0.15 | F1 | 1.5 | G1 | 2 | H1 | 1.2 | 0.6 | 100°C |
| Ex. 4 | S1 | A4 | 50 | B1 | 18 | C1 | 10 | D1 | 15 | E2 | 0.2 | F1 | 1.5 | G1 | 2.2 | H1 | 1.2 | 0,6 | 100°C |
| Ex. 5 | S1 | A5 | 50 | B1 | 15 | C1 | 11 | D1 | 15 | E2 | 0.25 | F1 | 1.5 | G1 | 2.5 | H1 | 1.2 | 0.6 | 100°C |
| Ex. 6 | S1 | A6 | 50 | B1 | 16 | C1 | 12 | D2 | 15 | E2 | 0.3 | F1 | 1.5 | G1 | 2.7 | H1 | 1.2 | 0.6 | 100°C |
| Ex. 7 | S1 | A7 | 50 | B1 | 17 | C1 | 7 | D2 | 15 | E2 | 0.35 | F1 | 2.5 | G1 | 3 | H1 | 1.2 | 0.6 | 100°C |
| Ex. 8 | S1 | A8 | 50 | B1 | 18 | C1 | 8 | D2 | 15 | E2 | 0.4 | F1 | 2.5 | G1 | 3.2 | H1 | 1.2 | 0.6 | 100°C |
| Ex. 9 | S1 | A9 | 50 | B1 | 19 | C1 | 9 | D2 | 15 | E2 | 0.45 | F1 | 2.5 | G1 | 3.5 | H1 | 1.2 | 0.6 | 100°C |
| Ex. 10 | S1 | A10 | 50 | B1 | 20 | C1 | 10 | D2 | 15 | E2 | 0.5 | F1 | 2.5 | G1 | 3.2 | H1 | 1.2 | 0.6 | 100°C |
| Ex. 11 | S1 | A11 | 50 | B1 | 21 | C1 | 11 | D3 | 15 | E5 | 0.4 | F1 | 2.5 | G1 | 3 | H1 | 1.2 | 0.6 | 100°C |
| Ex. 12 | S1 | A12 | 50 | B1 | 22 | C1 | 12 | D3 | 15 | E5 | 0.35 | F1 | 2.5 | G1 | 2.7 | H1 | 1.2 | 0.6 | 100°C |
| Ex. 13 | S1 | A13 | 50 | B1 | 23 | C1 | 7 | D3 | 15 | E5 | 0.3 | F1 | 3.5 | G1 | 3.5 | H1 | 1.2 | 0.6 | 100°C |
| Ex. 14 | S1 | A14 | 50 | B1 | 24 | C1 | 8 | D3 | 15 | E5 | 0.25 | F1 | 3.5 | G1 | 2.2 | H1 | 1.2 | 0.6 | 100°C |
| Ex. 15 | S1 | A15 | 50 | B1 | 25 | C1 | 9 | D3 | 15 | E5 | 0.2 | F1 | 3.5 | G1 | 2 | H1 | 1.2 | 0.6 | 100°C |
| Ex. 16 | S1 | A16 | 50 | B1 | 26 | C1 | 10 | D4 | 15 | E5 | 0.15 | F1 | 3.5 | G1 | 1.7 | H1 | 1.2 | 0.6 | 100°C |
| Ex. 17 | S1 | A17 | 50 | B1 | 27 | C1 | 11 | D4 | 15 | E5 | 0.1 | F1 | 3.5 | G1 | 1.5 | H1 | 1.2 | 0.6 | 100°C |
| Ex. 18 | S1 | A2 | 40 | B1 | 15 | C1 | 15 | D4 | 13 | E5 | 0.1 | F1 | 3.5 | G2 | 1 | H1 | 1 | 0.3 | 60°C |
| Ex. 19 | S1 | A2 | 50 | B4 | 20 | C5 | 8 | D4 | 17 | E5 | 0.3 | F2 | 1 | G2 | 2 | H2 | 2 | 0.6 | 70°C |
| Ex. 20 | S1 | A2 | 60 | B9 | 25 | C7 | 5 | D4 | 21 | E5 | 0.5 | F3 | 1.5 | G2 | 3 | H3 | 1.5 | 1.0 | 80°C |
| Ex. 21 | S1 | A5 | 40 | B1 | 15 | C1 | 15 | D5 | 13 | E1 | 0.1 | F1 | 2 | G2 | 1 | H4 | 1 | 0.3 | 90°C |
| Ex. 22 | S1 | A5 | 50 | B4 | 20 | C5 | 8 | D5 | 17 | E1 | 0.3 | F2 | 2.5 | G2 | 2 | H5 | 2 | 0.6 | 100°C |
| Ex. 23 | S1 | A5 | 60 | B9 | 25 | C7 | 5 | D5 | 21 | E1 | 0.5 | F3 | 3 | G2 | 3 | H6 | 1.5 | 1.0 | 120°C |
| Ex. 24 | S1 | A8 | 40 | B1 | 15 | C1 | 15 | D5 | 13 | E1 | 0.1 | F1 | 3.5 | G2 | 1 | H7 | 1 | 0.3 | 60°C |
| Ex. 25 | S1 | A8 | 50 | B4 | 20 | C5 | 8 | D5 | 17 | E1 | 0.3 | F2 | 4 | G2 | 2 | H1 | 2 | 0.6 | 70°C |
| Ex. 26 | S1 | A8 | 60 | B9 | 25 | C7 | 5 | D6 | 21 | E2 | 0.5 | F3 | 1 | G2 | 3 | H2 | 1.5 | 1.0 | 80°C |
| Ex. 27 | S1 | A9 | 40 | B1 | 15 | C1 | 15 | D6 | 13 | E2 | 0.1 | F1 | 1.5 | G2 | 1 | H3 | 1 | 0.3 | 90°C |
| Ex. 28 | S1 | A9 | 50 | B4 | 20 | C5 | 8 | D6 | 17 | E2 | 0.3 | F2 | 2 | G2 | 2 | H4 | 2 | 0.6 | 100°C |
| Ex. 29 | S1 | A9 | 60 | B9 | 25 | C7 | 5 | D6 | 21 | E2 | 0.5 | F3 | 2.5 | G2 | 3 | H5 | 1.5 | 1.0 | 120°C |
| Ex. 30 | S1 | A10 | 40 | B1 | 15 | C1 | 15 | D6 | 13 | E2 | 0.1 | F1 | 3 | G2 | I | H6 | 1 | 0.3 | 60°C |
| Ex. 31 | S1 | A10 | 50 | B4 | 20 | C5 | 8 | D1 | 17 | E4 | 0.3 | F2 | 3.5 | G2 | 2 | H7 | 2 | 0.6 | 70°C |
| Ex. 32 | S1 | A10 | 60 | B9 | 25 | C7 | 5 | D1 | 21 | E4 | 0.5 | F3 | 4 | G2 | 3 | H1 | 1.5 | 1.0 | 80°C |
| Ex. 33 | S1 | A11 | 40 | B1 | 15 | C1 | 15 | D1 | 13 | E4 | 0.1 | F1 | 1 | G2 | 1 | H2 | 1 | 0.3 | 90°C |
| Ex. 34 | S1 | A11 | 50 | B4 | 20 | C5 | 8 | D1 | 17 | E4 | 0.3 | F2 | 1.3 | G2 | 2 | H3 | 2 | 0.6 | 100°C |
| Ex. 35 | S1 | A11 | 60 | B9 | 25 | C7 | 5 | D1 | 21 | E4 | 0.5 | F3 | 1.5 | G2 | 3 | H4 | 1.5 | 1.0 | 120°C |
| Ex. 36 | S1 | A13 | 40 | B1 | 15 | C1 | 15 | D1 | 13 | E6 | 0.1 | F1 | 1.7 | G2 | 1 | H5 | 1 | 0.3 | 60°C |
| Ex. 37 | S1 | A13 | 50 | B4 | 20 | C5 | 8 | D1 | 17 | E6 | 0.3 | F2 | 1.9 | G2 | 2 | H6 | 2 | 0.6 | 70°C |
| Ex. 38 | S1 | A13 | 60 | B9 | 25 | C7 | 5 | D1 | 21 | E6 | 0.5 | F3 | 2.2 | G2 | 3 | H7 | 1.5 | 1.0 | 80°C |
| Ex. 39 | S1 | A15 | 40 | B1 | 15 | C1 | 15 | D1 | 13 | E6 | 0.1 | F1 | 2.5 | G2 | 1 | H1 | 1 | 0.3 | 90°C |
| Ex. 40 | S1 | A15 | 50 | B4 | 20 | C5 | 8 | D1 | 17 | E6 | 0.3 | F2 | 2.7 | G2 | 2 | H2 | 2 | 0.6 | 100°C |
| Ex. 41 | S1 | A15 | 60 | B9 | 25 | C7 | 5 | D4 | 21 | E3 | 0.5 | F3 | 3 | G3 | 3 | H3 | 1.5 | 1.0 | 120°C |
| Ex. 42 | S1 | A16 | 40 | B1 | 15 | C1 | 15 | D4 | 13 | E3 | 0.1 | F1 | 3.2 | G3 | 1 | H4 | 1 | 0.3 | 100°C |
| Ex. 43 | S1 | A16 | 50 | B4 | 20 | C5 | 8 | D4 | 17 | E3 | 0.3 | F2 | 3.5 | G3 | 2 | H5 | 2 | 0.6 | 100°C |
| Ex. 44 | S1 | A16 | 60 | B9 | 25 | C7 | 5 | D4 | 21 | E3 | 0.5 | F3 | 3.7 | G3 | 3 | H6 | 1.5 | 1.0 | 100°C |
| Ex. 45 | S1 | A2 | 40 | B1 | 30 | C2 | 15 | D4 | 10 | E3 | 0.05 | F2 | 1 | G3 | 0.5 | H7 | 0.1 | 0.6 | 100°C |
| Ex. 46 | S1 | A2 | 43 | B1 | 28 | C2 | 14 | D4 | 12 | E3 | 0.07 | F2 | 4 | G3 | 0.8 | H2 | 0.4 | 0.6 | 100°C |
| Ex. 47 | S1 | A2 | 45 | B1 | 26 | C2 | 13 | D4 | 14 | E3 | 0.1 | F2 | 1.4 | G3 | 1.1 | H2 | 0.7 | 0.6 | 100°C |
| Ex. 48 | S1 | A2 | 47 | B1 | 24 | C2 | 12 | D4 | 16 | E3 | 0.13 | F2 | 3.7 | G3 | 1.5 | H2 | 1 | 0.6 | 100°C |
| Ex. 49 | S1 | A2 | 50 | B1 | 22 | C2 | 11 | D4 | 18 | E3 | 0.15 | F2 | 1.8 | G3 | 1.8 | H2 | 1.3 | 0.6 | 100°C |
| Ex. 50 | S1 | A2 | 52 | B7 | 20 | C4 | 10 | D4 | 19 | E3 | 0.17 | F2 | 3.3 | G3 | 2.1 | H3 | 1.6 | 0.6 | 100°C |
| Ex. 51 | s1 | A2 | 55 | B7 | 17 | C4 | 9 | D2 | 20 | E3 | 0.2 | F2 | 2.2 | G3 | 2.4 | H3 | 1.9 | 0.6 | 100°C |
| Ex. 52 | S1 | A2 | 56 | B7 | 15 | C4 | 8 | D2 | 21 | E3 | 0.23 | F2 | 3 | G3 | 2.7 | H3 | 2.1 | 0.6 | 100°C |
| Ex. 53 | S1 | A2 | 58 | B7 | 13 | C4 | 7 | D2 | 23 | E3 | 0.25 | F2 | 2.5 | G3 | 3 | H3 | 2.3 | 0.6 | 100°C |
| Ex. 54 | S1 | A2 | 60 | B7 | 10 | C4 | 6 | D2 | 25 | E3 | 0.27 | F2 | 2.7 | G3 | 3.5 | H3 | 2.5 | 0.6 | 100°C |
| Ex. 55 | S1 | A11 | 41 | B4 | 11 | C3 | 5 | D2 | 25 | E3 | 0.15 | F2 | 3.8 | G3 | 1 | H4 | 0.1 | 0.6 | 100°C |
| Ex. 56 | S1 | A11 | 43 | B4 | 12 | C3 | 6 | D2 | 24 | E3 | 0.18 | F2 | 2.7 | G3 | 1.3 | H4 | 0.4 | 0.6 | 100°C |
| Ex. 57 | S1 | A11 | 44 | B4 | 14 | C3 | 7 | D2 | 22 | E3 | 0.23 | F2 | 1.9 | G3 | 1.7 | H4 | 0.7 | 0.6 | 100°C |
| Ex. 58 | S1 | A11 | 46 | B4 | 16 | C3 | 8 | D2 | 20 | E3 | 0.27 | F2 | 3.5 | G3 | 2 | H4 | 1 | 0.6 | 100°C |
| Ex. 59 | S1 | A11 | 48 | B4 | 18 | C3 | 9 | D2 | 18 | E3 | 0.3 | F2 | 2.4 | G3 | 2.3 | H4 | 1.3 | 0.6 | 100°C |
| Ex. 60 | S1 | A11 | 52 | B9 | 20 | C6 | 10 | D2 | 17 | E3 | 0.32 | F2 | 1.6 | G3 | 2.7 | H5 | 1.6 | 0.6 | 100°C |
| Ex. 61 | S1 | A11 | 54 | B9 | 22 | C6 | 11 | D5 | 16 | E3 | 0.35 | F2 | 3.3 | G1 | 3 | H5 | 1.9 | 0.6 | 100°C |
| Ex. 62 | S1 | A11 | 56 | B9 | 24 | C6 | 12 | D5 | 14 | E3 | 0.37 | F2 | 2.3 | G2 | 3.3 | H5 | 2.1 | 0.6 | 100°C |
| Ex. 63 | S1 | A11 | 58 | B9 | 26 | C6 | 13 | D5 | 12 | E3 | 0.4 | F2 | 1.4 | G3 | 3.6 | H5 | 2.3 | 0.6 | 100°C |
| Ex. 64 | S1 | A11 | 60 | B9 | 28 | C6 | 14 | D5 | 10 | E3 | 0.44 | F2 | 3.1 | G4 | 4 | H5 | 2.5 | 0.6 | 100°C |
| Ex. 65 | S1 | A16 | 40 | B2 | 21 | C8 | 15 | D5 | 18 | E3 | 0.3 | F4 | 2.1 | G1 | 3.7 | H6 | 0.1 | 0.6 | 100°C |
| Ex. 66 | S1 | A16 | 43 | B2 | 23 | C8 | 13 | D5 | 17 | E3 | 0.25 | F4 | 1.1 | G2 | 3.4 | H6 | 0.4 | 0.6 | 100°C |
| Ex. 67 | S1 | A16 | 45 | B2 | 25 | C8 | 12 | D5 | 16 | E3 | 0.2 | F4 | 2.1 | G3 | 3.1 | H6 | 0.7 | 0.6 | 100°C |
| Ex. 68 | S1 | A16 | 47 | B2 | 27 | C8 | 11 | D5 | 15 | E3 | 0.17 | F4 | 2.2 | G4 | 1.8 | H6 | 1 | 0.6 | 100°C |
| Ex. 69 | S1 | A16 | 50 | B2 | 29 | C8 | 10 | D5 | 14 | E3 | 0.15 | F4 | 2.5 | G1 | 1.5 | H6 | 1.3 | 0.6 | 100°C |
| Ex. 70 | S1 | A16 | 52 | B5 | 19 | C1 | 9 | D5 | 19 | E3 | 0.14 | F4 | 3.1 | G2 | 1.2 | H7 | 1.6 | 0.6 | 100°C |
| Ex. 71 | S1 | A16 | 55 | B5 | 18 | C1 | 8 | D1 | 20 | E4 | 0.12 | F4 | 2.7 | G3 | 2.9 | H7 | 1.9 | 0.6 | 100°C |
| Ex. 72 | S1 | A16 | 56 | B5 | 16 | C1 | 7 | D1 | 21 | E4 | 0.1 | F4 | 2.7 | G4 | 2.6 | H7 | 2.1 | 0.6 | 100°C |
| Ex. 73 | S1 | A16 | 58 | B5 | 14 | C1 | 6 | D1 | 22 | E4 | 0.07 | F4 | 2.7 | G1 | 2.3 | H7 | 2.3 | 0.6 | 100°C |
| Ex. 74 | S1 | A16 | 60 | B5 | 12 | C1 | 5 | D1 | 23 | E4 | 0.05 | F4 | 2.7 | G2 | 2 | H7 | 2.5 | 0.6 | 100°C |
| Ex. 75 | S1 | A17 | 40 | B6 | 14 | C1 | 7 | D1 | 10 | E4 | 0.1 | F1 | 2.7 | G3 | 1.5 | H7 | 1.4 | 0.6 | 100°C |
| Ex. 76 | S1 | A17 | 45 | B6 | 16 | C1 | 7.5 | D1 | 11 | E4 | 0.2 | F1 | 2.7 | G4 | 1.9 | H2 | 1.1 | 0.6 | 100°C |
| Ex. 77 | S1 | A17 | 50 | B6 | 18 | C1 | 8 | D1 | 12 | E4 | 0.3 | F1 | 2.7 | G1 | 2.9 | H2 | 1.1 | 0.6 | 100°C |
| Ex. 78 | S1 | A17 | 55 | B6 | 20 | C1 | 8.5 | D1 | 13 | E4 | 0.4 | F1 | 2.7 | G2 | 2.4 | H2 | 1.1 | 0.6 | 100°C |
| Ex. 79 | S1 | A17 | 60 | B6 | 22 | C1 | 9 | D1 | 14 | E4 | 0.5 | F1 | 2.7 | G3 | 3.3 | H2 | 1.1 | 0.6 | 100°C |
| Ex. 80 | S1 | A8 | 45 | B4 | 19 | C1 | 9.5 | D1 | 15 | E4 | 0.15 | F1 | 2.7 | G4 | 4 | H2 | 1.1 | 0.6 | 100°C |
| Ex. 81 | S1 | A9 | 47 | B4 | 21 | C1 | 10 | D1 | 16 | E4 | 0.25 | F1 | 2.7 | G1 | 3.5 | H2 | 1.1 | 0.6 | 100°C |
| Ex. 82 | S1 | A12 | 49 | B4 | 23 | C1 | 7.5 | D1 | 17 | E4 | 0.35 | F1 | 2.7 | G2 | 3.1 | H2 | 1.1 | 0.6 | 100°C |
| Ex. 83 | S1 | A14 | 50 | B4 | 25 | C1 | 8 | D1 | 20 | E4 | 0.45 | F1 | 2.7 | G3 | 2.8 | H2 | 1.1 | 0.6 | 100°C |
| Ex. 84 | S1 | A15 | 52 | B4 | 27 | C1 | 8.5 | D1 | 21 | E4 | 0.4 | F1 | 2.7 | G4 | 2.5 | H2 | 1.1 | 0.6 | 100°C |
| Ex. 85 | S1 | A16 | 55 | B4 | 29 | C1 | 9 | D1 | 23 | E4 | 0.35 | F1 | 2.7 | G1 | 1.5 | H2 | 1.1 | 0.6 | 100°C |
| Ex. 86 | S2 | A2 | 47 | B1 | 19 | C1 | 9.5 | D4 | 25 | E4 | 0.3 | F1 | 2.7 | G2 | 2.2 | H2 | 1.1 | 0.6 | 100°C |
| Ex. 87 | S2 | A8 | 49 | B1 | 17 | C1 | 10 | D4 | 20 | E4 | 0.25 | F1 | 2.7 | G3 | 3.2 | H2 | 1.1 | 0.6 | 100°C |
| Ex. 88 | S2 | A10 | 50 | B1 | 15 | C1 | 7.5 | D4 | 19 | E4 | 0.2 | F1 | 2.7 | G4 | 1.2 | H2 | 1.1 | 0.6 | 100°C |
| Ex. 89 | S2 | A11 | 52 | B1 | 13 | C1 | 8 | D4 | 18 | E4 | 0.15 | F1 | 2.7 | G1 | 1.6 | H2 | 1.1 | 0.6 | 100°C |
| Ex. 90 | S2 | A15 | 55 | B1 | 11 | C1 | 8.5 | D4 | 17 | E4 | 0.1 | F1 | 2.7 | G2 | 3.6 | H2 | 1.1 | 0.6 | 100°C |
| Ex. 91 | S3 | A2 | 47 | B1 | 18 | C1 | 9 | D4 | 16 | E4 | 0.15 | F1 | 2.7 | G3 | 2.6 | H2 | 1.1 | 0.6 | 100°C |
| Ex. 92 | S3 | A8 | 49 | B1 | 20 | C1 | 9.5 | D4 | 15 | E4 | 0.2 | F1 | 2.7 | G4 | 1.8 | H2 | 1.1 | 0.6 | 100°C |
| Ex. 93 | S3 | A10 | 50 | B1 | 22 | C1 | 10 | D4 | 14 | E4 | 0.25 | F1 | 2.7 | G1 | 2.2 | H2 | 1.1 | 0.6 | 100°C |
| Ex. 94 | S3 | A11 | 52 | B1 | 24 | C1 | 7.5 | D4 | 13 | E4 | 0.3 | F1 | 2.7 | G1 | 2.2 | H2 | 1.1 | 0.6 | 100°C |
| Ex. 95 | S3 | A15 | 55 | B1 | 26 | C1 | 8 | D4 | 12 | E4 | 0.35 | F1 | 2.7 | G1 | 2.2 | H2 | 1.1 | 0.6 | 100°C |
| Ex. 96 | S4 | A2 | 47 | B1 | 17 | C1 | 8.5 | D4 | 11 | E4 | 0.4 | F1 | 2.7 | G1 | 2.2 | H2 | 1.1 | 0.6 | 100°C |
| Ex. 97 | S4 | A8 | 49 | B1 | 16 | C1 | 9 | D4 | 10 | E4 | 0.45 | F1 | 2.7 | G1 | 2.2 | H2 | 1.1 | 0.6 | 100°C |
| Ex. 98 | S4 | A10 | 50 | B1 | 15 | C1 | 9.5 | D4 | 15 | E4 | 0.5 | F1 | 2.7 | G1 | 2.2 | H2 | 1.1 | 0.6 | 100°C |
| Ex. 99 | S4 | A11 | 52 | B1 | 14 | C1 | 10 | D4 | 20 | E4 | 0.4 | F1 | 2.7 | G1 | 2.2 | H2 | 1.1 | 0.6 | 100°C |

| Ex. 100 | S4 | A15 | 55 | B1 | 13 | C1 | 7.5 | D4 | 25 | E4 | 0.3 | F1 | 2.7 | G1 | 2.2 | H2 | 1.1 | 0.6 | 100°C |
|---|---|---|---|---|---|---|---|---|---|---|---|---|---|---|---|---|---|---|---|
| Comp. Ex. 1 | S1 | A2 | 40 | - | - | C1 | 6 | D1 | 15 | E3 | 0.1 | F1 | 1.5 | G1 | 3.5 | H1 | 1.5 | 0.4 | 100°C |
| Comp. Ex. 2 | S1 | A8 | 45 | B1 | 16 | - | - | D1 | 20 | E3 | 0.2 | F1 | 2 | G1 | 3 | H1 | 1.5 | 0.4 | 100°C |
| Comp. Ex. 3 | S1 | A10 | 50 | B3 | 18 | C2 | 8 | - | - | E3 | 0.3 | F1 | 2.5 | G1 | 2.5 | H1 | 1.5 | 0.5 | 100°C |
| Comp. Ex. 4 | S1 | A11 | 55 | B4 | 20 | C3 | 10 | D1 | 25 | - | - | F1 | 3 | G1 | 2 | H1 | 1.5 | 0.5 | 100°C |
| Comp. Ex. 5 | S1 | A15 | 60 | B7 | 22 | C4 | 12 | D1 | 10 | E3 | 0.4 | - | - | G1 | 1.5 | H1 | 1.5 | 0.6 | 100°C |
| Comp. Ex. 6 | S1 | A2 | 40 | - | - | C5 | 6 | D5 | 17 | E4 | 0.4 | F2 | 1.5 | G3 | 1 | H2 | 2 | 0.6 | 100°C |
| Comp. Ex. 7 | S1 | A8 | 45 | B1 | 16 | - | - | D5 | 18 | E4 | 0.3 | F2 | 2 | G3 | 2 | H2 | 2 | 0.7 | 100°C |
| Comp. Ex. 8 | S1 | A10 | 50 | B3 | 18 | C6 | 8 | - | - | E4 | 0.2 | F2 | 2.5 | G3 | 3 | H2 | 2 | 0.7 | 100°C |
| Comp. Ex. 9 | S1 | A11 | 55 | B4 | 20 | C7 | 10 | D5 | 21 | - | - | F2 | 3 | G3 | 4 | H2 | 2 | 0.8 | 100°C |
| Comp. Ex. 10 | S1 | A15 | 60 | B7 | 22 | C8 | 12 | D5 | 22 | E4 | 0.1 | F2 | 3.5 | - | - | H2 | 2 | 0.8 | 100°C |
| Comp. Ex. 11 | S1 | A2 | 40 | B1 | 25 | C1 | 15 | D1 | 15 | E1 | 0.2 | F1 | 2.5 | G1 | 2 | H1 | 1.2 | 0.2 | 100°C |
| Comp. Ex. 12 | S1 | A8 | 45 | B1 | 22 | C1 | 12 | D2 | 17 | E2 | 0.2 | F2 | 2.5 | G2 | 2 | H2 | 1.2 | 0.5 | 50°C |
| Comp. Ex. 13 | S1 | A10 | 50 | B3 | 19 | C2 | 9 | D3 | 19 | E3 | 0.2 | F3 | 2.5 | G3 | 2 | H3 | 1.2 | 1.5 | 100°C |
| Comp. Ex. 14 | S1 | A11 | 55 | B4 | 17 | C3 | 7 | D4 | 21 | E4 | 0.2 | F4 | 2.5 | G1 | 2 | H4 | 1.2 | 0.7 | 150°C |
| Comp. Ex. 15 | S1 | A15 | 60 | B7 | 15 | C4 | 5 | D5 | 23 | E5 | 0.2 | F1 | 2.5 | G3 | 2 | H5 | 1.2 | 1.2 | 100°C |

### (3) Evaluation tests

After coated with the aqueous inorganic surface treatment agents for the test sample sheets in the above Examples 1-100 and Comparative Examples 1-15, the test sample sheets were sampled and tested according to the following testing methods, and the tested data for evaluating the various properties thereof were obtained and listed in Table 11. The tests for evaluating the various property parameters thereof are described as follows:
1) Corrosion resistance of flat sheets:
   A salt spray test was performed on a flat sheet. The test standard was ASTMB117, and the test time was 120 hours. The evaluation criteria were:
   ⊚: White rust area ratio was less than 5%
   ○: White rust area ratio was greater than 5% and less than 10%
   Δ: White rust area ratio was greater than 10% and less than 50%
   ×: White rust area ratio was greater than 50%
2) Corrosion resistance after forming:
   8 mm cupping was performed using an Erichson cupping instrument, and a salt spray test was performed on the cupped portion. The test standard was ASTM B117, and the test time was 72 hours. The evaluation criteria were:
   ⊚ : White rust area ratio on the cupped portion was less than 5%
   ○: White rust area ratio on the cupped portion was greater than 5% and less than 10%
   Δ: White rust area ratio on the cupped portion was greater than 10% and less than 50%
   ×: White rust area ratio on the cupped portion was greater than 50%
3) Resistance to red rust corrosion:
   A salt spray test was performed on a flat sheet. The test standard was ASTMB117, and the time when red rust began to appear was recorded. The evaluation criteria were:
   ⊚: The time when red rust began to appear on S1 steel sheets was more than 240 hours; the time when red rust began to appear on S2-S4 steel sheets was more than 288 hours
   ○: The time when red rust began to appear on S1 steel sheets was more than 196 hours but less than 240 hours; the time when red rust began to appear on S2-S4 steel sheets was more than 240 hours but less than 288 hours
   Δ: The time when red rust began to appear on S1 steel sheets was more than 168 hours but less than 196 hours; the time when red rust began to appear on S2-S4 steel sheets was more than 196 hours but less than 240 hours
   ×: The time when red rust began to appear on S1 steel sheets was less than 168 hours; the time when red rust began to appear on S2-S4 steel sheets was less than 196 hours
4) Stamping formability:
   A drawbead method was used to prepare samples. Experimental conditions: fixed under-bead pressure 3KN, indenter diameter 9.6mm, drawing speed 200mm/min, evaluation criteria:
   ⊚: The appearance had no change.
   ○: The appearance had a small amount of black spots.
   Δ: The appearance had a relatively large amount of obvious black streaks.
   ×: The appearance was completely blackened.
5) "Non-stick" property of skin film surfaces:
   A drawbead method was used to prepare samples. Experimental conditions: fixed under-bead pressure 7 KN, indenter diameter 9.6 mm, and drawing speed 200 mm/min. After the drawing test was completed, the surfaces of the sample sheets were blown with a hair dryer for 5 seconds, and then the cleanness of the surfaces of the sample sheets was observed. Evaluation criteria:
   ⊚: No skin film chippings or zinc powder adhered to the surface
   ○: A trace amount of skin film chippings and zinc powder adhered to the surface
   Δ: Some skin film chippings and zinc powder adhered to the surface
   ×: A large amount of skin film chippings and zinc powder adhered to the surface
6) Wear resistance:
   A rubber abrasion method was utilized with a load of 500g, a stroke distance of 20mm and a speed of 300mm/min. The abrasion was repeated for 50 times. Evaluation criteria:
   ⊚: No change in the skin film
   ○: A small amount of scratches on the skin film
   Δ: A plurality of scratches on the skin film
   ×: The skin film fell off completely
7) Surface electric conductivity:
   Surface resistance values of the upper and lower surfaces were measured using a four-needle method, wherein 10 points were measured on the upper and lower surfaces. An average surface resistance value at the 20 points was calculated. Evaluation criteria:
   ⊚: The average surface resistance value was less than 0.1 milliohms.
   ○: The average surface resistance value was greater than 0.1 milliohms and less than 0.5 milliohms.
   Δ: The average surface resistance value was greater than 0.5 milliohms and less than 1 milliohm.
   ×: The average surface resistance value was greater than 1 milliohm.
8) Coatability:
   The surface-treated galvanized steel sheets were coated under the following conditions, and then the coating adhesion test was carried out. The test conditions were as follows:
   Ink (Japan Seiko Ink), 14# bar coating, baking conditions: baking at 120 °C for 20 minutes;
   After application of the above two coatings, an art knife was used to scribe 100 small lattices in a surface of a coating film, wherein the lattice size was 1 mm², and the depth should reach the surface of the steel sheet by cutting through the paint film layer. After peeling off with a glass cloth tape, the number of the residual lattices of the paint film was counted. A larger number of residual lattices indicated better coatability of the steel sheet for the ink.

**Table 11: Various properties of the test sample sheets**

| No. | Corrosion resistance of flat sheet | Corrosion resistance after forming | Red rust resistance | Stamping formability: | "Non-stick" property of surface | Wear resistance: | Surface electric conductivity: | Coatability |
|---|---|---|---|---|---|---|---|---|
| Ex. 1 | ○ | ○ | ○ | ⊚ | ○ | ⊚ | ○ | ⊚ |
| Ex. 2 | ○ | ○ | ○ | ⊚ | ○ | ⊚ | ○ | ⊚ |
| Ex. 3 | ○ | ○ | ○ | ⊚ | ○ | ⊚ | ○ | ⊚ |
| Ex. 4 | ⊚ | ⊚ | ⊚ | ⊚ | ○ | ⊚ | ⊚ | ⊚ |
| Ex. 5 | ⊚ | ⊚ | ⊚ | ⊚ | ○ | ⊚ | ⊚ | ⊚ |
| Ex. 6 | ⊚ | ⊚ | ⊚ | ⊚ | ○ | ⊚ | ⊚ | ⊚ |
| Ex. 7 | ○ | ○ | ○ | ⊚ | ○ | ⊚ | ⊚ | ⊚ |
| Ex. 8 | ○ | ○ | ○ | ⊚ | ○ | ⊚ | ⊚ | ⊚ |
| Ex. 9 | ○ | ○ | ○ | ⊚ | ○ | ⊚ | ⊚ | ⊚ |
| Ex. 10 | ⊚ | ⊚ | ⊚ | ⊚ | ⊚ | ○ | ⊚ | ○ |
| Ex. 11 | ⊚ | ⊚ | ⊚ | ⊚ | ⊚ | ○ | ⊚ | ○ |
| Ex. 12 | ⊚ | ⊚ | ⊚ | ⊚ | ⊚ | ○ | ⊚ | ○ |
| Ex. 13 | ⊚ | ⊚ | ⊚ | ⊚ | ⊚ | ○ | ⊚ | ○ |
| Ex. 14 | ⊚ | ⊚ | ⊚ | ⊚ | ⊚ | ○ | ⊚ | ⊚ |
| Ex. 15 | ⊚ | ⊚ | ⊚ | ⊚ | ⊚ | ○ | ⊚ | ⊚ |
| Ex. 16 | ⊚ | ⊚ | ⊚ | ⊚ | ⊚ | ○ | ○ | ⊚ |
| Ex. 17 | ⊚ | ⊚ | ⊚ | ⊚ | ⊚ | ○ | ○ | ⊚ |
| Ex. 18 | ○ | ○ | ○ | ⊚ | ○ | ⊚ | ○ | ⊚ |
| Ex. 19 | ⊚ | ⊚ | ⊚ | ⊚ | ○ | ⊚ | ⊚ | ⊚ |
| Ex. 20 | ⊚ | ⊚ | ⊚ | ○ | ○ | ⊚ | ⊚ | ⊚ |
| Ex. 21 | ○ | ○ | ○ | ⊚ | ○ | ⊚ | ○ | ⊚ |
| Ex. 22 | ⊚ | ⊚ | ⊚ | ⊚ | ○ | ⊚ | ⊚ | ⊚ |
| Ex. 23 | ⊚ | ⊚ | ⊚ | ○ | ○ | ⊚ | ⊚ | ⊚ |
| Ex. 24 | ○ | ○ | ○ | ⊚ | ○ | ⊚ | ○ | ⊚ |
| Ex. 25 | ⊚ | ⊚ | ⊚ | ⊚ | ○ | ⊚ | ⊚ | ⊚ |
| Ex. 26 | ⊚ | ⊚ | ⊚ | ○ | ○ | ⊚ | ⊚ | ⊚ |
| Ex. 27 | ○ | ○ | ○ | ⊚ | ○ | ⊚ | ○ | ⊚ |
| Ex. 28 | ⊚ | ⊚ | ⊚ | ⊚ | ○ | ⊚ | ⊚ | ⊚ |
| Ex. 29 | ⊚ | ⊚ | ⊚ | ○ | ○ | ⊚ | ⊚ | ⊚ |
| Ex. 30 | ○ | ○ | ○ | ⊚ | ⊚ | ⊚ | ○ | ○ |
| Ex. 31 | ⊚ | ⊚ | ⊚ | ⊚ | ⊚ | ⊚ | ⊚ | Δ |
| Ex. 32 | ⊚ | ⊚ | ⊚ | ○ | ⊚ | ○ | ⊚ | ○ |
| Ex. 33 | ○ | ○ | ○ | ⊚ | ⊚ | ⊚ | ○ | ○ |
| Ex. 34 | ⊚ | ⊚ | ⊚ | ⊚ | ⊚ | ⊚ | ⊚ | Δ |
| Ex. 35 | ⊚ | ⊚ | ⊚ | ○ | ⊚ | ○ | ⊚ | ○ |
| Ex. 36 | ○ | ○ | ○ | ⊚ | ⊚ | ⊚ | ○ | ○ |
| Ex. 37 | ⊚ | ⊚ | ⊚ | ⊚ | ⊚ | ⊚ | ⊚ | Δ |
| Ex. 38 | ⊚ | ⊚ | ⊚ | ○ | ⊚ | ○ | ⊚ | ○ |
| Ex. 39 | ○ | ○ | ○ | ⊚ | ⊚ | ⊚ | ○ | ○ |
| Ex. 40 | ⊚ | ⊚ | ⊚ | ⊚ | ⊚ | ⊚ | ⊚ | Δ |
| Ex. 41 | ⊚ | ⊚ | ⊚ | ○ | ⊚ | ○ | ⊚ | ○ |
| Ex. 42 | ○ | ○ | ○ | ⊚ | ⊚ | ⊚ | ○ | ○ |
| Ex. 43 | ⊚ | ⊚ | ⊚ | ⊚ | ⊚ | ⊚ | ⊚ | Δ |
| Ex. 44 | ⊚ | ⊚ | ⊚ | ○ | ⊚ | ○ | ⊚ | ○ |
| Ex. 45 | ⊚ | ⊚ | ⊚ | ○ | ○ | ⊚ | Δ | ⊚ |
| Ex. 46 | ⊚ | ⊚ | ⊚ | ○ | ○ | ⊚ | Δ | ⊚ |
| Ex. 47 | ⊚ | ⊚ | ⊚ | ⊚ | ○ | ⊚ | ○ | ⊚ |
| Ex. 48 | ⊚ | ⊚ | ⊚ | ⊚ | ○ | ⊚ | ○ | ⊚ |
| Ex. 49 | ⊚ | ⊚ | ⊚ | ⊚ | ○ | ⊚ | ○ | ⊚ |
| Ex. 50 | ⊚ | ⊚ | ⊚ | ⊚ | ○ | ⊚ | ○ | ⊚ |
| Ex. 51 | ⊚ | ⊚ | ⊚ | ⊚ | ○ | ⊚ | ⊚ | ⊚ |
| Ex. 52 | ○ | ○ | ○ | ⊚ | ○ | ⊚ | ⊚ | ⊚ |
| Ex. 53 | ○ | ○ | ○ | ⊚ | ○ | ⊚ | ⊚ | ⊚ |
| Ex. 54 | ○ | ○ | ○ | ⊚ | ○ | ⊚ | ⊚ | ⊚ |
| Ex. 55 | ○ | ○ | ○ | ⊚ | ⊚ | ⊚ | ○ | Δ |
| Ex. 56 | ○ | ○ | ○ | ⊚ | ⊚ | ⊚ | ○ | Δ |
| Ex. 57 | ⊚ | ⊚ | ⊚ | ⊚ | ⊚ | ⊚ | ⊚ | ○ |
| Ex. 58 | ⊚ | ⊚ | ⊚ | ⊚ | ⊚ | ⊚ | ⊚ | ○ |
| Ex. 59 | ⊚ | ⊚ | ⊚ | ⊚ | ⊚ | ○ | ⊚ | ○ |
| Ex. 60 | ⊚ . | ⊚ | ⊚ | ⊚ | ⊚ | ○ | ⊚ | ○ |
| Ex. 61 | ⊚ | ⊚ | ⊚ | ⊚ | ⊚ | ○ | ⊚ | ○ |
| Ex. 62 | ⊚ | ⊚ | ⊚ | ⊚ | ⊚ | ○ | ⊚ | ○ |
| Ex. 63 | ⊚ | ⊚ | ⊚ | ○ | ⊚ | ○ | ⊚ | ○ |
| Ex. 64 | ⊚ | ⊚ | ⊚ | ○ | ⊚ | ○ | ⊚ | ○ |
| Ex. 65 | ⊚ | ⊚ | ⊚ | ⊚ | ⊚ | ○ | ⊚ | Δ |
| Ex. 66 | ⊚ | ⊚ | ⊚ | ⊚ | ⊚ | ○ | ⊚ | Δ |
| Ex. 67 | ⊚ | ⊚ | ⊚ | ⊚ | ⊚ | ○ | ⊚ | ○ |
| Ex. 68 | ⊚ | ⊚ | ⊚ | ⊚ | ⊚ | ○ | ○ | ○ |
| Ex. 69 | ⊚ | ⊚ | ⊚ | ⊚ | ⊚ | ○ | ○ | ○ |
| Ex. 70 | ⊚ | ⊚ | ⊚ | ⊚ | ⊚ | ○ | ○ | ○ |
| Ex. 71 | ⊚ | ⊚ | ⊚ | ⊚ | ⊚ | ⊚ | ○ | ○ |
| Ex. 72 | ⊚ | ⊚ | ⊚ | ⊚ | ⊚ | ⊚ | ○ | ○ |
| Ex. 73 | ○ | ○ | ○ | ⊚ | ⊚ | ⊚ | Δ | ○ |
| Ex. 74 | ○ | ○ | ○ | ⊚ | ⊚ | ⊚ | Δ | ○ |
| Ex. 75 | ○ | ○ | ○ | ○ | ⊚ | ○ | ○ | ○ |
| Ex. 76 | ⊚ | ⊚ | ⊚ | ○ | ⊚ | ○ | ⊚ | ○ |
| Ex. 77 | ⊚ | ⊚ | ⊚ | ○ | ⊚ | ○ | ⊚ | ○ |
| Ex. 78 | ⊚ | ⊚ | ⊚ | ⊚ | ⊚ | ○ | ⊚ | ○ |
| Ex. 79 | ⊚ | ⊚ | ⊚ | ⊚ | ⊚ | ○ | ⊚ | ○ |
| Ex. 80 | ⊚ | ⊚ | ⊚ | ⊚ | ○ | ⊚ | ⊚ | ⊚ |
| Ex. 81 | ⊚ | ⊚ | ⊚ | ⊚ | ○ | ⊚ | ⊚ | ⊚ |
| Ex. 82 | ⊚ | ⊚ | ⊚ | ⊚ | ⊚ | ○ | ⊚ | ○ |
| Ex. 83 | ⊚ | ⊚ | ⊚ | ⊚ | ⊚ | ⊚ | ⊚ | ○ |
| Ex. 84 | ⊚ | ⊚ | ⊚ | ⊚ | ⊚ | ⊚ | ⊚ | ○ |
| Ex. 85 | ⊚ | ⊚ | ⊚ | ⊚ | ○ | ⊚ | ⊚ | Δ |
| Ex. 86 | ⊚ | ⊚ | ⊚ | ⊚ | ○ | ⊚ | ⊚ | ⊚ |
| Ex. 87 | ○ | ○ | ○ | ⊚ | ⊚ | ⊚ | ⊚ | ⊚ |
| Ex. 88 | ○ | ○ | ○ | ⊚ | ⊚ | ○ | ⊚ | ○ |
| Ex. 89 | ○ | ○ | ○ | ⊚ | ⊚ | ○ | ○ | ○ |
| Ex. 90 | ○ | ○ | ○ | ⊚ | ○ | ○ | ○ | ○ |
| Ex. 91 | ⊚ | ⊚ | ⊚ | ⊚ | ○ | ⊚ | ⊚ | ⊚ |
| Ex. 92 | ⊚ | ⊚ | ⊚ | ⊚ | ⊚ | ⊚ | ⊚ | ⊚ |
| Ex. 93 | ⊚ | ⊚ | ⊚ | ⊚ | ⊚ | ○ | ⊚ | ○ |
| Ex. 94 | ⊚ | ⊚ | ⊚ | ⊚ | ⊚ | ○ | ⊚ | ○ |
| Ex. 95 | ⊚ | ⊚ | ⊚ | ○ | ⊚ | ○ | ⊚ | ○ |
| Ex. 96 | ⊚ | ⊚ | ⊚ | ○ | ○ | ⊚ | ⊚ | ⊚ |
| Ex. 97 | ⊚ | ⊚ | ⊚ | ○ | ○ | ⊚ | ⊚ | ⊚ |
| Ex. 98 | ⊚ | ⊚ | ⊚ | ⊚ | ⊚ | ⊚ | ⊚ | ○ |
| Ex. 99 | ⊚ | ⊚ | ⊚ | ⊚ | ⊚ | ⊚ | ⊚ | Δ |
| Ex. 100 | ⊚ | ⊚ | ⊚ | ⊚ | ⊚ | ⊚ | ⊚ | Δ |
| Comp. Ex. 1 | Δ | Δ | Δ | ⊚ | ○ | ⊚ | ○ | ⊚ |
| Comp. Ex. 2 | Δ | Δ | Δ | ⊚ | ○ | ⊚ | ○ | ○ |
| Comp. Ex. 3 | ⊚ | ⊚ | ⊚ | × | ⊚ | × | ⊚ | ⊚ |
| Comp. Ex. 4 | ○ | ○ | ○ | ○ | ⊚ | ○ | × | Δ |
| Comp. Ex. 5 | ○ | ○ | Δ | ○ | ⊚ | ○ | ⊚ | ⊚ |
| Comp. Ex. 6 | Δ | Δ | Δ | ○ | ○ | ○ | ⊚ | ⊚ |
| Comp. Ex. 7 | ○ | ○ | Δ | ○ | ○ | Δ | ○ | ○ |
| Comp. Ex. 8 | ⊚ | ⊚ | ⊚ | × | ○ | × | ⊚ | ○ |
| Comp. Ex. 9 | Δ | Δ | Δ | ⊚ | ⊚ | ⊚ | × | ○ |
| Comp. Ex. 10 | Δ | Δ | Δ | ⊚ | ⊚ | ⊚ | ○ | ○ |
| Comp. Ex. 11 | Δ | Δ | × | × | ○ | × | ⊚ | ⊚ |
| Comp. Ex. 12 | Δ | Δ | × | × | ○ | × | ○ | Δ |
| Comp. Ex. 13 | ⊚ | ⊚ | ⊚ | ○ | ⊚ | ○ | × | Δ |
| Comp. Ex. 14 | Δ | Δ | Δ | Δ | ⊚ | Δ | Δ | Δ |
| Comp. Ex. 15 | ○ | ○ | ⊚ | ○ | ⊚ | ⊚ | × | Δ |

Table 11 lists the tested various property parameters of the test sample sheets coated with the aqueous inorganic surface treatment agents in Examples 1-100 and Comparative Examples 1-15.

As can be seen from Table 11, after the test sample sheets coated with the aqueous inorganic surface treatment agents in Example 1-100 were tested, an overwhelming majority of the Examples each showed an evaluation result of "⊚" or "O", except for a small number of Examples that showed "Δ" in a certain evaluation result, indicating that the galvanized steel sheets coated with the aqueous inorganic surface treatment agent of the present disclosure all have excellent red rust resistance, surface electric conductivity, surface lubricating property and resistance to blackening caused by stamping, and can meet the requirements of rapid deep-drawing processing with progressive dies and bare service.

As can be seen from Tables 10 and 11 in combination, in contrast to Example 1-100, the corrosion resistance of the inorganic skin films in Comparative Example 1, Comparative Example 2, Comparative Example 6 and Comparative Example 7 was poor due to the low crosslinking density of the inorganic skin films caused by the absence of the systematic crosslinking agent (C) or the water-soluble nanosol (C) in the aqueous inorganic surface treatment agents.

The aqueous inorganic surface treatment agents in Comparative Example 3 and Comparative Example 8 did not contain surface-modified high-density polyethylene particles (D). Therefore, the stamping formability and wear resistance of the inorganic skin films of the galvanized steel sheets coated with these aqueous inorganic surface treatment agents were poor.

The aqueous inorganic surface treatment agents in Comparative Example 4 and Comparative Example 9 did not contain an orthosilicate-modified graphene oxide (E), and a conductive network could not be formed in the inorganic skin films. Therefore, the electric conductivity of the galvanized steel sheets coated with these aqueous inorganic surface treatment agents was poor. In addition, since the inorganic skin film thicknesses of Comparative Example 13 and Comparative Example 15 were relatively large, the surface electric conductivity was also poor.

The aqueous inorganic surface treatment agents in Comparative Example 5 and Comparative Example 10 did not contain the water-soluble fluorine-containing compound (F) or the water-soluble phosphorus-containing compound (G), so that the corrosion resistance of the inorganic skin films was poor.

The thickness of the inorganic skin film in Comparative Example 11 was small, resulting in poor overall performance. In Comparative Example 12, the baking and curing temperature was low, resulting in an inorganic skin film that was not completely cured, so that the inorganic skin film was inferior in overall performance.

It is to be noted that there are listed above only specific examples of the invention. Obviously, the present disclosure is not limited to the above examples.

## Claims

1. An inorganically surface-treated galvanized steel sheet, wherein the inorganically surface-treated galvanized steel sheet is a galvanized steel sheet having a surface coated with a single-layer inorganic skin film having a dry film thickness of 0.3-1.0 µm, wherein the inorganic skin film comprises:
A) one or more hydrophobic monoorganosilane coupling agents in an amount of 40-60 parts by weight of the inorganic skin film;
wherein the hydrophobic monoorganosilane coupling agent comprises X hydrophobic groups (X is 1 or 2) and 4-X reactive groups;
B) a systematic crosslinking agent in an amount of 10-30 parts by weight of the inorganic skin film;
wherein the systematic crosslinking agent is one or more of an orthosilicate, a titanate or a diorganosilane coupling agent having a bridging structure;
C) a water-soluble nanosol in an amount of 5-15 parts by weight of the inorganic skin film;
wherein the water-soluble nanosol has a mass fraction of 20-30%;
D) surface-modified high-density polyethylene particles in an amount of 10-25 parts by weight of the inorganic skin film;
E) an orthosilicate-modified graphene oxide, wherein the graphene oxide is 0.05-0.5 parts by weight of the inorganic skin film;
wherein the orthosilicate-modified graphene oxide is a dark brown n-propanol suspension, wherein the orthosilicate-modified graphene oxide has a mass fraction of 1-5%.

2. The inorganically surface-treated galvanized steel sheet according to claim 1, wherein the inorganic skin film further comprises:
F) a water-soluble fluorine-containing compound, wherein fluorine element is 1-4 parts by weight of the inorganic skin film;
G a water-soluble phosphorus-containing compound, wherein phosphorus element is 0.5-4 parts by weight of the inorganic skin film;
H) a water-soluble metal salt compound, wherein metal element is 0.1-2.5 parts by weight of the inorganic skin film.

3. The inorganically surface-treated galvanized steel sheet according to claim 1, wherein the hydrophobic group in the hydrophobic monoorganosilane coupling agent (A) is one or two selected from the group consisting of -CH3 (methyl), -C2H5 (ethyl), -C3H7 (propyl), -C6H5 (phenyl), -CF3 (perfluoromethyl), -C2F5 (perfluoroethyl), -C3F7 (perfluoropropyl), -C5F11 (perfluoropentyl), -C7F15 (perfluoroheptyl) and -C9F19 (perfluorononyl).

4. The inorganically surface-treated galvanized steel sheet according to claim 1, wherein the reactive group in the hydrophobic monoorganosilane coupling agent is one to three selected from the group consisting of -OCH3 (methoxy), -OC2H5 (ethoxy), vinyl, propenyl, epoxy, amino, hydroxyl, carboxyl, amido and 2,3-epoxypropoxy.

5. The inorganically surface-treated galvanized steel sheet according to claim 1, wherein a sum of the number of the hydrophobic groups and the number of the reactive groups in the hydrophobic monoorganosilane coupling agent is equal to four;
the hydrophobic monoorganosilane coupling agent is 40-60 parts by weight, preferably 45-55 parts by weight of the inorganic skin film.

6. A method of preparing the inorganically surface-treated galvanized steel sheet of any one of claims 1-5, wherein forming an aqueous inorganic surface treatment agent by dissolving or dispersing components of the aqueous inorganic surface treatment agent in water, applying the aqueous inorganic surface treatment agent on a surface of a galvanized steel sheet by one-pass roll coating, and drying at 60-100 °C, thereby providing an inorganic skin film having a dry film thickness of 0.3-1.0 µm,
wherein the inorganic skin film comprises:
A) one or more hydrophobic monoorganic silane coupling agents in an amount of 40-60 parts by weight of the inorganic skin film;
wherein the hydrophobic monoorganosilane coupling agent comprises X hydrophobic groups (X is 1 or 2) and 4-X reactive groups;
B) a systematic crosslinking agent in an amount of 10-30 parts by weight of the inorganic skin film;
wherein the systematic crosslinking agent is one or more selected from an orthosilicate, a titanate or a diorganosilane coupling agent having a bridging structure;
C) a water-soluble nanosol in an amount of 5-15 parts by weight of the inorganic skin film;
wherein the water-soluble nanosol has a mass fraction of 20-30%;
D) surface-modified high-density polyethylene particles in an amount of 10-25 parts by weight of the inorganic skin film;
E) an orthosilicate-modified graphene oxide, wherein the graphene oxide is 0.05-0.5 parts by weight of the inorganic skin film;
wherein the orthosilicate-modified graphene oxide is a dark brown n-propanol suspension, wherein the orthosilicate-modified graphene oxide has a mass fraction of 1-5%.

7. The method of preparing the inorganically surface-treated galvanized steel sheet according to claim 6, wherein the inorganic skin film further comprises:
F) a water-soluble fluorine-containing compound, wherein fluorine element is 1-4 parts by weight of the inorganic skin film;
G) a water-soluble phosphorus-containing compound, wherein phosphorus element is 0.5-4 parts by weight of the inorganic skin film;
H) a water-soluble metal salt compound, wherein metal element is 0.1-2.5 parts by weight of the inorganic skin film.

8. The method of preparing the inorganically surface-treated galvanized steel sheet according to claim 6, preferably
the hydrophobic group in the hydrophobic monoorganosilane coupling agent (A) is one or two of -CH3 (methyl), -C2H5 (ethyl), -C3H7 (propyl), -C6H5 (phenyl), - CF3 (perfluoromethyl), -C2F5 (perfluoroethyl), -C3F7 (perfluoropropyl), -C5F11 (perfluoropentyl), -C7F15 (perfluoroheptyl) or -C9F19 (perfluorononyl); the reactive group in the hydrophobic monoorganosilane coupling agent is at most three of -OCH3 (methoxy), -OC2H5 (ethoxy), vinyl, propenyl, epoxy, amino, hydroxyl, carboxyl, amido or 2,3-epoxypropoxy; a sum of the number of the hydrophobic groups and the number of the reactive groups in the hydrophobic monoorganosilane coupling agent is equal to four; the hydrophobic monoorganosilane coupling agent is 40-60 parts by weight, preferably 45-55 parts by weight of the inorganic skin film.

9. The method of preparing the inorganically surface-treated galvanized steel sheet according to claim 6, wherein the systematic cross-linking agent (B) is one or more of an orthosilicate having 4 reactive groups, a titanate having 4 reactive groups or a diorganosilane coupling agent having 6 reactive groups and a bridging structure; the reactive group in the orthosilicate is any one of a methoxy group, an ethoxy group, a propoxy group or a butoxy group; the reactive group in the titanate is one or more of an isopropyl ester group, a phosphoryloxy group, a benzenesulfonyloxy group or a n-butyl ester group; the bridging structure of the diorganosilane coupling agent is consisting of 2-4 methylene groups, amino groups or 2-4 mercapto groups; the reactive group of the diorganosilane coupling agent is any one of a methoxy group, an ethoxy group or a propoxy group.

10. An aqueous inorganic surface treatment agent for surface treatment of a galvanized steel sheet by coating a surface of the galvanized steel sheet to form an inorganic skin film by the method of any one of claims 6-9, wherein total solids in an aqueous solution thereof comprise the following components:
A) one or more hydrophobic monoorganosilane coupling agents in an amount of 40-60 parts by weight of the inorganic skin film;
wherein the hydrophobic monoorganosilane coupling agent comprises X hydrophobic groups (X is 1 or 2) and 4-X reactive groups;
B) a systematic crosslinking agent in an amount of 10-30 parts by weight of the inorganic skin film;
wherein the systematic crosslinking agent is one or more of an orthosilicate, a titanate or a diorganosilane coupling agent having a bridging structure;
C) a water-soluble nanosol in an amount of 5-15 parts by weight of the inorganic skin film;
wherein the water-soluble nanosol has a mass fraction of 20-30%;
D) surface-modified high-density polyethylene particles in an amount of 10-25 parts by weight of the inorganic skin film;
E) an orthosilicate-modified graphene oxide, wherein the graphene oxide is 0.05-0.5 parts by weight of the inorganic skin film;
wherein the orthosilicate-modified graphene oxide is a dark brown n-propanol suspension, wherein the orthosilicate-modified graphene oxide has a mass fraction of 1-5%;
F) a water-soluble fluorine-containing compound, wherein fluorine element is 1-4 parts by weight of the inorganic skin film;
G) a water-soluble phosphorus-containing compound, wherein phosphorus element is 0.5-4 parts by weight of the inorganic skin film;
H) a water-soluble metal salt compound, wherein metal element is 0.1-2.5 parts by weight of the inorganic skin film.

11. The aqueous inorganic surface treatment agent for surface treatment of a galvanized steel plate according to claim 10, wherein the hydrophobic group in the hydrophobic monoorganosilane coupling agent (A) is one or two of -CH3 (methyl), -C2H5 (ethyl), -C3H7 (propyl), -C6H5 (phenyl), -CF3 (perfluoromethyl), -C2F5 (perfluoroethyl), -C3F7 (perfluoropropyl), -C5F11 (perfluoropentyl), -C7F15 (perfluoroheptyl) or -C9F19 (perfluorononyl); the reactive group in the hydrophobic monoorganosilane coupling agent is at most three of -OCH3 (methoxy), -OC2H5 (ethoxy), vinyl, propenyl, epoxy, amino, hydroxyl, carboxyl, amido or 2,3-epoxypropoxy; a sum of the number of the hydrophobic groups and the number of the reactive groups in the hydrophobic monoorganosilane coupling agent is equal to four; the hydrophobic monoorganosilane coupling agent is 40-60 parts by weight, preferably 45-55 parts by weight of the inorganic skin film.

12. The aqueous inorganic surface treatment agent for surface treatment of a galvanized steel plate according to claim 10, wherein the systematic cross-linking agent (B) is one or more selected from the group consisting of an orthosilicate having 4 reactive groups, a titanate having 4 reactive groups and a diorganosilane coupling agent having 6 reactive groups and a bridging structure; the reactive group in the orthosilicate is any one selected from the group consisting of a methoxy group, an ethoxy group, a propoxy group and a butoxy group; the reactive group in the titanate is one or more selected from the group consisting of an isopropyl ester group, a phosphoryloxy group, a benzenesulfonyloxy group and a n-butyl ester group; the bridging structure of the diorganosilane coupling agent is consisting of 2-4 methylene groups, amino groups or 2-4 mercapto groups; the reactive group of the diorganosilane coupling agent is any one selected from the group consisting of a methoxy group, an ethoxy group and a propoxy group.

## Patentansprüche

1. Anorganisch oberflächenbehandeltes verzinktes Stahlblech, wobei das anorganisch oberflächenbehandelte verzinkte Stahlblech ein verzinktes Stahlblech mit einer Oberfläche ist, die mit einer einschichtigen anorganischen Hautschicht mit einer Trockenfilmdicke von 0,3-1,0 µm beschichtet ist, wobei die anorganische Hautschicht aufweist:
A) ein oder mehrere wasserabweisende monoorganosilane Haftmittel in einer Menge von 40-60 Gewichtsteilen der anorganischen Hautschicht;
wobei das wasserabweisende monoorganosilane Haftmittel X wasserabweisende Gruppen (X ist 1 oder 2) und 4-X reaktionsfreudige Gruppen aufweist;
B) ein systematisches Vernetzungsmittel in einer Menge von 10-30 Gewichtsteilen der anorganischen Hautschicht;
wobei das systematische Vernetzungsmittel ein oder mehrere von einem Orthosilikat, einem Titanat oder einem diorganosilanen Haftmittel mit einer Überbrückungsstruktur ist;
C) ein wasserlösliches Nanosol in einer Menge von 5-15 Gewichtsteilen der anorganischen Hautschicht;
wobei das wasserlösliche Nanosol einen Massenanteil von 20-30 % aufweist;
D) oberflächenmodifizierte Polyethylenpartikel mit hoher Dichte in einer Menge von 10-25 Gewichtsteilen der anorganischen Hautschicht;
E) ein orthosilikatmodifiziertes Graphenoxid, wobei das Graphenoxid 0,05-0,5 Gewichtsteile der anorganischen Hautschicht ist;
wobei das orthosilikatmodifizierte Graphenoxid eine dunkelbraune n-Propanol-Suspension ist, wobei das orthosilikatmodifizierte Graphenoxid einen Massenanteil von 1-5 % aufweist.

2. Anorganisch oberflächenbehandeltes verzinktes Stahlblech nach Anspruch 1, wobei die anorganische Hautschicht ferner aufweist:
F) eine wasserlösliche fluorhaltige Verbindung, wobei ein Fluorelement 1-4 Gewichtsteile der anorganischen Hautschicht ist;
G) eine wasserlösliche phosphorhaltige Verbindung, wobei ein Phosphorelement 0,5-4 Gewichtsteile der anorganischen Hautschicht ist;
H) eine wasserlösliche Metallsalzverbindung, wobei ein Metallelement 0,1-2,5 Gewichtsteile der anorganischen Hautschicht ist.

3. Anorganisch oberflächenbehandeltes verzinktes Stahlblech nach Anspruch 1, wobei die wasserabweisende Gruppe im wasserabweisenden monoorganosilanen Haftmittel (A) eines oder zwei ausgewählt aus der Gruppe, die aus -CH3(Methyl), -C2H5 (Ethyl), -C3H7 (Propyl), -C6H5 (Phenyl), -CF3 (Perfluoromethyl), -C2F5 (Perfluoroethyl), -C3F7 (Perfluoropropyl), -C5F11 (Perfluoropentyl), -C7F15 (Perfluoroheptyl) und -C9F19 (Perfluorononyl) besteht, ist.

4. Anorganisch oberflächenbehandeltes verzinktes Stahlblech nach Anspruch 1, wobei die reaktionsfreudige Gruppe im wasserabweisenden monoorganosilanen Haftmittel eines oder drei ausgewählt aus der Gruppe, die aus -OCH3 (Methoxy), -OC2H5 (Ethoxy), Vinyl, Propenyl, Epoxid, Amino, Hydroxyl, Carboxyl, Amido und 2,3-Epoxidpropoxy besteht, ist.

5. Anorganisch oberflächenbehandeltes verzinktes Stahlblech nach Anspruch 1, wobei eine Summe der Anzahl der wasserabweisenden Gruppen und der Anzahl der reaktionsfreudigen Gruppen im wasserabweisenden monoorganosilanen Haftmittel gleich 4 ist;
wobei das wasserabweisende monoorganosilane Haftmittel 40-60 Gewichtsteile, bevorzugt 45-55 Gewichtsteile, der anorganischen Hautschicht ist.

6. Verfahren zum Herstellen des anorganisch oberflächenbehandelten verzinkten Stahlblechs nach einem der Ansprüche 1-5, wobei ein wässriges anorganisches Oberflächenbehandlungsmittel durch Auflösen oder Dispergieren von Komponenten des wässrigen anorganischen Oberflächenbehandlungsmittels in Wasser ausgebildet wird, das wässrige anorganische Oberflächenbehandlungsmittel durch Einpass-Walzenbeschichten auf eine Oberfläche des verzinkten Stahlblechs angewandt wird und bei 60-100 °C getrocknet wird, wodurch eine anorganische Hautschicht mit einer Trockenfilmdicke von 0,3-1,0 µm vorgesehen wird,
wobei die anorganische Hautschicht aufweist:
A) ein oder mehrere wasserabweisende monoorganosilane Haftmittel in einer Menge von 40-60 Gewichtsteilen der anorganischen Hautschicht;
wobei das wasserabweisende monoorganosilane Haftmittel X wasserabweisende Gruppen (X ist 1 oder 2) und 4-X reaktionsfreudige Gruppen aufweist;
B) ein systematisches Vernetzungsmittel in einer Menge von 10-30 Gewichtsteilen der anorganischen Hautschicht;
wobei das systematische Vernetzungsmittel ein oder mehrere von einem Orthosilikat, einem Titanat oder einem diorganosilanen Haftmittel mit einer Überbrückungsstruktur ist;
C) ein wasserlösliches Nanosol in einer Menge von 5-15 Gewichtsteilen der anorganischen Hautschicht;
wobei das wasserlösliche Nanosol einen Massenanteil von 20-30 % aufweist;
D) oberflächenmodifizierte Polyethylenpartikel mit hoher Dichte in einer Menge von 10-25 Gewichtsteilen der anorganischen Hautschicht;
E) ein orthosilikatmodifiziertes Graphenoxid, wobei das Graphenoxid 0,05-0,5 Gewichtsteile der anorganischen Hautschicht ist;
wobei das orthosilikatmodifizierte Graphenoxid eine dunkelbraune n-Propanol-Suspension ist, wobei das orthosilikatmodifizierte Graphenoxid einen Massenanteil von 1-5 % aufweist.

7. Verfahren zum Herstellen des anorganisch oberflächenbehandelten verzinkten Stahlblechs nach Anspruch 6, wobei die anorganische Hautschicht ferner aufweist:
F) eine wasserlösliche fluorhaltige Verbindung, wobei ein Fluorelement 1-4 Gewichtsteile der anorganischen Hautschicht ist;
G) eine wasserlösliche phosphorhaltige Verbindung, wobei ein Phosphorelement 0,5-4 Gewichtsteile der anorganischen Hautschicht ist;
H) eine wasserlösliche Metallsalzverbindung, wobei ein Metallelement 0,1-2,5 Gewichtsteile der anorganischen Hautschicht ist.

8. Verfahren zum Herstellen des anorganisch oberflächenbehandelten verzinkten Stahlblechs nach Anspruch 6, wobei bevorzugt wird, dass
die wasserabweisende Gruppe im wasserabweisenden monoorganosilanen Haftmittel (A) eines oder zwei von -CH3(Methyl), -C2H5 (Ethyl), -C3H7 (Propyl), -C6H5 (Phenyl), -CF3 (Perfluoromethyl), -C2F5 (Perfluoroethyl), - C3F7 (Perfluoropropyl), -C5F11 (Perfluoropentyl), -C7F15 (Perfluoroheptyl) und -C9F19 (Perfluorononyl) ist; die reaktionsfreudige Gruppe im wasserabweisenden monoorganosilanen Haftmittel höchstens drei von -OCH3 (Methoxy), -OC2H5 (Ethoxy), Vinyl, Propenyl, Epoxid, Amino, Hydroxyl, Carboxyl, Amido oder 2,3-Epoxidpropoxy ist; eine Summe der Anzahl der wasserabweisenden Gruppen und der Anzahl der reaktionsfreudigen Gruppen im wasserabweisenden monoorganosilanen Haftmittel gleich 4 ist; das wasserabweisende monoorganosilane Haftmittel 40-60 Gewichtsteile, bevorzugt 45-55 Gewichtsteile, der anorganischen Hautschicht ist.

9. Verfahren zum Herstellen des anorganisch oberflächenbehandelten verzinkten Stahlblechs nach Anspruch 6, wobei das systematische Vernetzungsmittel (B) ein oder mehrere von einem Orthosilikat mit 4 reaktionsfreudigen Gruppen, einem Titanat mit 4 reaktionsfreudigen Gruppen oder einem diorganosilanen Haftmittel mit 6 reaktionsfreudigen Gruppen und einer Überbrückungsstruktur ist; die reaktionsfreudige Gruppe im Orthosilikat jegliche einer Methoxygruppe, einer Ethoxygruppe, einer Propoxygruppe oder einer Butoxygruppe ist; die reaktionsfreudige Gruppe im Titanat eine oder mehrere von einer Isopropylestergruppe, einer Phosphoryloxygruppe, einer Benzenesulfonyloxygruppe oder einer n-Butylestergruppe ist; die Überbrückungsstruktur des diorganosilanen Haftmittels aus 2-4 Methylengruppen, Aminogruppen oder 2-4 Mercaptogruppen besteht; die reaktionsfreudige Gruppe des diorganosilanen Haftmittels jegliche einer Methoxygruppe, einer Ethoxygruppe oder einer Propoxygruppe ist.

10. Wässriges anorganisches Oberflächenbehandlungsmittel zur Oberflächenbehandlung eines verzinkten Stahlblechs durch Beschichten einer Oberfläche des verzinkten Stahlblechs zur Ausbildung einer anorganischen Hautschicht durch das Verfahren nach einem der Ansprüche 6-9, wobei Gesamtfeststoffe in einer wässrigen Lösung davon die folgenden Komponenten aufweisen:
A) ein oder mehrere wasserabweisende monoorganosilane Haftmittel in einer Menge von 40-60 Gewichtsteilen der anorganischen Hautschicht;
wobei das wasserabweisende monoorganosilane Haftmittel X wasserabweisende Gruppen (X ist 1 oder 2) und 4-X reaktionsfreudige Gruppen aufweist;
B) ein systematisches Vernetzungsmittel in einer Menge von 10-30 Gewichtsteilen der anorganischen Hautschicht;
wobei das systematische Vernetzungsmittel ein oder mehrere von einem Orthosilikat, einem Titanat oder einem diorganosilanen Haftmittel mit einer Überbrückungsstruktur ist;
C) ein wasserlösliches Nanosol in einer Menge von 5-15 Gewichtsteilen der anorganischen Hautschicht;
wobei das wasserlösliche Nanosol einen Massenanteil von 20-30 % aufweist;
D) oberflächenmodifizierte Polyethylenpartikel mit hoher Dichte in einer Menge von 10-25 Gewichtsteilen der anorganischen Hautschicht;
E) in orthosilikatmodifiziertes Graphenoxid, wobei das Graphenoxid 0,05-0,5 Gewichtsteile der anorganischen Hautschicht ist;
wobei das orthosilikatmodifizierte Graphenoxid eine dunkelbraune n-Propanol-Suspension ist, wobei das orthosilikatmodifizierte Graphenoxid einen Massenanteil von 1-5 % aufweist;
F) eine wasserlösliche fluorhaltige Verbindung, wobei ein Fluorelement 1-4 Gewichtsteile der anorganischen Hautschicht ist;
G) eine wasserlösliche phosphorhaltige Verbindung, wobei ein Phosphorelement 0,5-4 Gewichtsteile der anorganischen Hautschicht ist;
H) eine wasserlösliche Metallsalzverbindung, wobei ein Metallelement 0,1-2,5 Gewichtsteile der anorganischen Hautschicht ist.

11. Wässriges anorganisches Oberflächenbehandlungsmittel zur Oberflächenbehandlung eines verzinkten Stahlblechs nach Anspruch 10, wobei die wasserabweisende Gruppe im wasserabweisenden monoorganosilanen Haftmittel (A) eines oder zwei von -CH3(Methyl), -C2H5 (Ethyl), -C3H7 (Propyl), -C6H5 (Phenyl), -CF3 (Perfluoromethyl), -C2F5 (Perfluoroethyl), - C3F7 (Perfluoropropyl), -C5F11 (Perfluoropentyl), -C7F15 (Perfluoroheptyl) und -C9F19 (Perfluorononyl) ist; die reaktionsfreudige Gruppe im wasserabweisenden monoorganosilanen Haftmittel höchstens drei von -OCH3 (Methoxy), -OC2H5 (Ethoxy), Vinyl, Propenyl, Epoxid, Amino, Hydroxyl, Carboxyl, Amido oder 2,3-Epoxidpropoxy ist; eine Summe der Anzahl der wasserabweisenden Gruppen und der Anzahl der reaktionsfreudigen Gruppen im wasserabweisenden monoorganosilanen Haftmittel gleich 4 ist; das wasserabweisende monoorganosilane Haftmittel 40-60 Gewichtsteile, bevorzugt 45-55 Gewichtsteile, der anorganischen Hautschicht ist.

12. Wässriges anorganisches Oberflächenbehandlungsmittel zur Oberflächenbehandlung eines verzinkten Stahlblechs nach Anspruch 10, wobei das systematische Vernetzungsmittel (B) ein oder mehrere ausgewählt aus einer Gruppe, die aus einem Orthosilikat mit 4 reaktionsfreudigen Gruppen, einem Titanat mit 4 reaktionsfreudigen Gruppen und einem diorganosilanen Haftmittel mit 6 reaktionsfreudigen Gruppen und einer Überbrückungsstruktur besteht, ist; die reaktionsfreudige Gruppe im Orthosilikat jegliche ausgewählt aus der Gruppe, die aus einer Methoxygruppe, einer Ethoxygruppe, einer Propoxygruppe oder einer Butoxygruppe besteht, ist; die reaktionsfreudige Gruppe im Titanat eine oder mehrere ausgewählt aus der Gruppe, die aus einer Isopropylestergruppe, einer Phosphoryloxygruppe, einer Benzenesulfonyloxygruppe oder einer n-Butylestergruppe besteht, ist; die Überbrückungsstruktur des diorganosilanen Haftmittels aus 2-4 Methylengruppen, Aminogruppen oder 2-4 Mercaptogruppen besteht; die reaktionsfreudige Gruppe des diorganosilanen Haftmittels jegliche ausgewählt aus der Gruppe, die aus einer Methoxygruppe, einer Ethoxygruppe oder einer Propoxygruppe besteht, ist.

## Revendications

1. Tôle d'acier galvanisée inorganiquement traitée en surface, où la tôle d'acier galvanisée inorganiquement traitée en surface est une tôle d'acier galvanisée ayant une surface revêtue avec un film de peau inorganique monocouche ayant une épaisseur de film sec de 0,3-1,0 µm, où le film de peau inorganique comprend :
A) un ou plusieurs agents de couplage de monoorganosilanes hydrophobes dans une quantité de 40-60 parties en masse du film de peau inorganique ;
où l'agent de couplage de monoorganosilane hydrophobe comprend X groupes hydrophobes (X est 1 ou 2) et 4-X groupes réactifs ;
B) un agent de réticulation systématique dans une quantité de 10-30 parties en masse du film de peau inorganique ;
où l'agent de réticulation systématique est un ou plusieurs d'un orthosilicate, un titanate ou un agent de couplage de diorganosilane ayant une structure de pontage ;
C) un nanosol soluble dans l'eau dans une quantité de 5-15 parties en masse du film de peau inorganique ;
où le nanosol soluble dans l'eau présente une fraction de masse de 20-30 % ;
D) des particules de polyéthylène haute densité modifiées en surface dans une quantité de 10-25 parties en masse du film de peau inorganique ;
E) un oxyde de graphène modifié par un orthosilicate, où l'oxyde de graphène est 0,05-0,5 partie en masse du film de peau inorganique ;
où l'oxyde de graphène modifié par un orthosilicate est une suspension de n-propanol brun foncé, où l'oxyde de graphène modifié par un orthosilicate présente une fraction de masse de 1-5 %.

2. Tôle d'acier galvanisée inorganiquement traitée en surface selon la revendication 1, où le film de peau inorganique comprend de plus :
F) un composé contenant du fluor soluble dans l'eau, où l'élément de fluor est 1-4 parties en masse du film de peau inorganique ;
G) un composé contenant du phosphore soluble dans l'eau, où l'élément de phosphore est 0,5-4 parties en masse du film de peau inorganique ;
H) un composé de sel de métal soluble dans l'eau, où l'élément de métal est 0,1-2,5 parties en masse du film de peau inorganique.

3. Tôle d'acier galvanisée inorganiquement traitée en surface selon la revendication 1, où le groupe hydrophobe dans l'agent de couplage de monoorganosilane hydrophobe (A) est un ou deux choisis dans le groupe consistant en -CH3 (méthyle), -C2H5 (éthyle), -C3H7 (propyle), -C6H5 (phényle), -CF3 (perfluorométhyle), -C2F5 (perfluoroéthyle), -C3F7 (perfluropropyle), -C5F11 (perfluoropentyle), -C7F15 (perfluoroheptyle) et -C9F19 (perfluorononyle).

4. Tôle d'acier galvanisée inorganiquement traitée en surface selon la revendication 1, où le groupe réactif dans l'agent de couplage de monoorganosilane hydrophobe est un à trois choisis dans le groupe consistant en -OCH3 (méthoxy), -OC2H5 (éthoxy), vinyle, propényle, époxy, amino, hydroxyle, carboxyle, amido et 2,3-époxypropoxy.

5. Tôle d'acier galvanisée inorganiquement traitée en surface selon la revendication 1, où une somme du nombre des groupes hydrophobes et du nombre des groupes réactifs dans l'agent de couplage de monoorganosilane hydrophobe est égale à quatre ;
l'agent de couplage de monoorganosilane hydrophobe est de 40-60 parties en masse, de préférence 45-55 parties en masse du film de peau inorganique.

6. Procédé de préparation de la tôle d'acier galvanisée inorganiquement traitée en surface selon l'une quelconque des revendications 1-5, où la formation d'un agent de traitement de surface inorganique aqueux par dissolution ou dispersion de constituants de l'agent de traitement de surface inorganique aqueux dans de l'eau, l'application de l'agent de traitement de surface inorganique aqueux sur une surface d'une tôle d'acier galvanisée par revêtement au rouleau en un passage, et séchage à 60-100°C, fournissant par-là un film de peau inorganique ayant une épaisseur de film sec de 0,3-1,0 µm,
où le film de peau inorganique comprend :
A) un ou plusieurs agents de couplage de monoorganosilanes hydrophobes dans une quantité de 40-60 parties en masse du film de peau inorganique ;
où l'agent de couplage de monoorganosilane hydrophobe comprend X groupes hydrophobes (X est 1 ou 2) et 4-X groupes réactifs ;
B) un agent de réticulation systématique dans une quantité de 10-30 parties en masse du film de peau inorganique ;
où l'agent de réticulation systématique est un ou plusieurs choisis parmi un orthosilicate, un titanate ou un agent de couplage de diorganosilane ayant une structure de pontage ;
C) un nanosol soluble dans l'eau dans une quantité de 5-15 parties en masse du film de peau inorganique ;
où le nanosol soluble dans l'eau présente une fraction de masse de 20-30 % ;
D) des particules de polyéthylène haute densité modifiées en surface dans une quantité de 10-25 parties en masse du film de peau inorganique ;
E) un oxyde de graphène modifié par un orthosilicate, où l'oxyde de graphène est 0,05-0,5 partie en masse du film de peau inorganique ;
où l'oxyde de graphène modifié par un orthosilicate est une suspension de n-propanol brun foncé, où l'oxyde de graphène modifié par un orthosilicate présente une fraction de masse de 1-5 %.

7. Procédé de préparation de la tôle d'acier galvanisée inorganiquement traitée en surface selon la revendication 6, où le film de peau inorganique comprend de plus :
F) un composé contenant du fluor soluble dans l'eau, où l'élément de fluor est 1-4 parties en masse du film de peau inorganique ;
G) un composé contenant du phosphore soluble dans l'eau, où l'élément de phosphore est 0,5-4 parties en masse du film de peau inorganique ;
H) un composé de sel de métal soluble dans l'eau, où l'élément de métal est 0,1-2,5 parties en masse du film de peau inorganique.

8. Procédé de préparation de la tôle d'acier galvanisée inorganiquement traitée en surface selon la revendication 6, de préférence le groupe hydrophobe dans l'agent de couplage de monoorganosilane hydrophobe (A) est un ou deux de -CH3 (méthyle), -C2H5 (éthyle), -C3H7 (propyle), -C6H5 (phényle), -CF3 (perfluorométhyle), -C2F5 (perfluoroéthyle), -C3F7 (perfluropropyle), -C5F11 (perfluoropentyle), -C7F15 (perfluoroheptyle) et -C9F19 (perfluorononyle) ; le groupe réactif dans l'agent de couplage de monoorganosilane hydrophobe est au plus trois de -OCH3 (méthoxy), -OC2H5 (éthoxy), vinyle, propényle, époxy, amino, hydroxyle, carboxyle, amido et 2,3-époxypropoxy ; une somme du nombre des groupes hydrophobes et du nombre des groupes réactifs dans l'agent de couplage de monoorganosilane hydrophobe est égale à quatre ; l'agent de couplage de monoorganosilane hydrophobe est 40-60 parties en masse, de préférence 45-55 parties en masse du film de peau inorganique.

9. Procédé de préparation de la tôle d'acier galvanisée inorganiquement traitée en surface selon la revendication 6, où l'agent de réticulation systématique (B) est un ou plusieurs d'un orthosilicate ayant 4 groupes réactifs, un titanate ayant 4 groupes réactifs ou un agent de couplage de diorganosilane ayant 6 groupes réactifs et une structure de pontage ; le groupe réactif dans l'orthosilicate est l'un quelconque d'un groupe méthoxy, un groupe éthoxy, un groupe propoxy ou un groupe butoxy ; le groupe réactif dans le titanate est un ou plusieurs d'un groupe ester isopropylique, un groupe phosphoryloxy, un groupe benzènesulfonyloxy ou un groupe ester n-butylique ; la structure de pontage de l'agent de couplage de diorganosilane consiste en 2-4 groupes méthylène, groupes amino ou 2-4 groupes mercapto ; le groupe réactif de l'agent de couplage de diorganosilane est l'un quelconque d'un groupe méthoxy, un groupe éthoxy ou un groupe propoxy.

10. Agent de traitement de surface inorganique aqueux pour un traitement de surface d'une tôle d'acier galvanisée par revêtement d'une surface de la tôle d'acier galvanisée pour former un film de peau inorganique par le procédé selon l'une quelconque des revendications 6-9, où le total des solides dans une solution aqueuse de celui-ci comprend les constituants suivants :
A) un ou plusieurs agents de couplage de monoorganosilanes hydrophobes dans une quantité de 40-60 parties en masse du film de peau inorganique ;
où l'agent de couplage de monoorganosilane hydrophobe comprend X groupes hydrophobes (X est 1 ou 2) et 4-X groupes réactifs ;
B) un agent de réticulation systématique dans une quantité de 10-30 parties en masse du film de peau inorganique ;
où l'agent de réticulation systématique est un ou plusieurs d'un orthosilicate, un titanate ou un agent de couplage de diorganosilane ayant une structure de pontage ;
C) un nanosol soluble dans l'eau dans une quantité de 5-15 parties en masse du film de peau inorganique ;
où le nanosol soluble dans l'eau présente une fraction de masse de 20-30 % ;
D) des particules de polyéthylène haute densité modifiées en surface dans une quantité de 10-25 parties en masse du film de peau inorganique ;
E) un oxyde de graphène modifié par un orthosilicate, où l'oxyde de graphène est 0,05-0,5 partie en masse du film de peau inorganique ;
où l'oxyde de graphène modifié par un orthosilicate est une suspension de n-propanol brun foncé, où l'oxyde de graphène modifié par un orthosilicate présente une fraction de masse de 1-5 % ;
F) un composé contenant du fluor soluble dans l'eau, où l'élément de fluor est 1-4 parties en masse du film de peau inorganique ;
G) un composé contenant du phosphore soluble dans l'eau, où l'élément de phosphore est 0,5-4 parties en masse du film de peau inorganique ;
H) un composé de sel de métal soluble dans l'eau, où l'élément de métal est 0,1-2,5 parties en masse du film de peau inorganique.

11. Agent de traitement de surface inorganique aqueux pour un traitement de surface d'une plaque d'acier galvanisée selon la revendication 10, où le groupe hydrophobe dans l'agent de couplage de monoorganosilane hydrophobe (A) est un ou deux de -CH3 (méthyle), -C2H5 (éthyle), -C3H7 (propyle), -C6H5 (phényle), -CF3 (perfluorométhyle), -C2F5 (perfluoroéthyle), -C3F7 (perfluropropyle), -C5F11 (perfluoropentyle), -C7F15 (perfluoroheptyle) et -C9F19 (perfluorononyle) ; le groupe réactif dans l'agent de couplage de monoorganosilane hydrophobe est au plus trois de -OCH3 (méthoxy), -OC2H5 (éthoxy), vinyle, propényle, époxy, amino, hydroxyle, carboxyle, amido ou 2,3-époxypropoxy ; une somme du nombre des groupes hydrophobes et du nombre des groupes réactifs dans l'agent de couplage de monoorganosilane hydrophobe est égale à quatre ; l'agent de couplage de monoorganosilane hydrophobe est 40-60 parties en masse, de préférence 45-55 parties en masse du film de peau inorganique.

12. Agent de traitement de surface inorganique aqueux pour un traitement de surface d'une plaque d'acier galvanisée selon la revendication 10, où l'agent de réticulation systématique (B) est un ou plusieurs choisis dans le groupe consistant en un orthosilicate ayant 4 groupes réactifs, un titanate ayant 4 groupes réactifs et un agent de couplage de diorganosilane ayant 6 groupes réactifs et une structure de pontage ; le groupe réactif dans l'orthosilicate est l'un quelconque choisi dans le groupe consistant en un groupe méthoxy, un groupe éthoxy, un groupe propoxy et un groupe butoxy ; le groupe réactif dans le titanate est un ou plusieurs choisis dans le groupe consistant en un groupe ester isopropylique, un groupe phosphoryloxy, un groupe benzènesulfonyloxy et un groupe ester n-butylique ; la structure de pontage de l'agent de couplage de diorganosilane consiste en 2-4 groupes méthylène, groupes amino ou 2-4 groupes mercapto ; le groupe réactif de l'agent de couplage de diorganosilane est l'un quelconque choisi dans un groupe consistant en un groupe méthoxy, un groupe éthoxy et un groupe propoxy.
